



US005672451A

**United States Patent** [19]**Tam et al.****[11] Patent Number:** **5,672,451****[45] Date of Patent:** **Sep. 30, 1997****[54] MIGRATION IMAGING MEMBERS**

[75] Inventors: **Man C. Tam; Liqin Chen; Edward G. Zwart; Daniel Bihon**, all of Mississauga; **Marie-Eve Perron**, Montreal, all of Canada

[73] Assignee: **Xerox Corporation**, Stamford, Conn.

[21] Appl. No.: **630,296**

[22] Filed: **Apr. 11, 1996**

[51] Int. Cl. <sup>6</sup> ..... **G03G 17/10**

[52] U.S. Cl. ..... **430/41; 430/49**

[58] Field of Search ..... **430/58, 64, 96, 430/41, 49**

**[56] References Cited****U.S. PATENT DOCUMENTS**

|           |        |                 |       |        |
|-----------|--------|-----------------|-------|--------|
| 4,464,450 | 8/1984 | Teuscher        | ..... | 430/59 |
| 4,933,244 | 6/1990 | Teuscher et al. | ..... | 430/96 |
| 5,102,756 | 4/1992 | Vincett et al.  | ..... | 430/41 |
| 5,215,838 | 6/1993 | Tam et al.      | ..... | 430/41 |

*Primary Examiner*—John Goodrow

*Attorney, Agent, or Firm*—Judith L. Byorick

**[57] ABSTRACT**

Disclosed is a migration imaging member which comprises (a) a substrate, (b) a conductive layer comprising indium tin oxide dispersed in a polymeric binder, (c) a siloxane film charge blocking layer comprising a hydrolysis reaction product of a silane of the formula



wherein  $R_1$  is an alkylidene group,  $R_2$  and  $R_3$  are each, independent of the other, a hydrogen atom, an alkyl group, a phenyl group, or a poly(ethyleneamino) group, and  $R_4$ ,  $R_5$ , and  $R_6$  are each, independent of the others, alkyl groups, said siloxane having reactive hydroxyl and ammonium groups attached to silicon atoms, and (d) a softenable layer comprising a softenable material and a photosensitive migration marking material. Optionally an antistatic layer comprising indium tin oxide dispersed in a polymeric binder is situated on the surface of the substrate spaced from the softenable layer.

**23 Claims, 1 Drawing Sheet**



FIG. 1



FIG. 2



FIG. 3

## **BACKGROUND OF THE INVENTION**

The present invention is directed to migration imaging members. One embodiment of the present invention is directed to a migration imaging member which comprises (a) a substrate, (b) a conductive layer comprising indium tin oxide dispersed in a polymeric binder, (c) a siloxane film charge blocking layer comprising a hydrolysis reaction product of a silane of the formula



wherein  $R_1$  is an alkylidene group,  $R_2$  and  $R_3$  are each, independent of the other, a hydrogen atom, an alkyl group, a phenyl group, or a poly(ethyleneamino) group, and  $R_4$ ,  $R_5$ , and  $R_6$  are each, independent of the others, alkyl groups, said siloxane having reactive hydroxyl and ammonium groups attached to silicon atoms, and (d) a softenable layer comprising a softenable material and a photosensitive migration marking material. Optionally an antistatic layer comprising indium tin oxide dispersed in a polymeric binder is situated on the surface of the substrate spaced from the softenable layer.

Migration imaging systems capable of producing high quality images of high optical contrast density and high resolution have been developed. Such migration imaging systems are disclosed in, for example, U.S. Pat. Nos. 5,215,838, 5,202,206, 5,102,756, 5,021,308, 4,970,130, 4,937,163, 4,883,731, 4,880,715, 4,853,307, 4,536,458, 4,536,457, 4,496,642, 4,482,622, 4,281,050, 4,252,890, 4,241,156, 4,230,782, 4,157,259, 4,135,926, 4,123,283, 4,102,682, 4,101,321, 4,084,966, 4,081,273, 4,078,923, 4,072,517, 4,065,307, 4,062,680, 4,055,418, 4,040,826, 4,029,502, 4,028,101, 4,014,695, 4,013,462, 4,012,250, 4,009,028, 4,007,042, 3,998,635, 3,985,560, 3,982,939, 3,982,936, 3,979,210, 3,976,483, 3,975,739, 3,975,195, and 3,909,262, the disclosures of each of which are totally incorporated herein by reference, and in "Migration Imaging Mechanisms, Exploitation, and Future Prospects of Unique Photographic Technologies, XDM and AMEN", P. S. Vincett, G. J. Kovacs, M. C. Tam, A. L. Pundsack, and P. H. Soden, *Journal of Imaging Science* 30 (4) July/August, pp. 183-191 (1986), the disclosure of which is totally incorporated herein by reference.

The expression "softenable" as used herein is intended to mean any material which can be rendered more permeable, thereby enabling particles to migrate through its bulk. Conventionally, changing the permeability of such material or reducing its resistance to migration of migration marking material is accomplished by dissolving, swelling, melting, or softening, by techniques, for example, such as contacting with heat, vapors, partial solvents, solvent vapors, solvents, and combinations thereof, or by otherwise reducing the viscosity of the softenable material by any suitable means.

The expression "fracturable" layer or material as used herein means any layer or material which is capable of breaking up during development, thereby permitting portions of the layer to migrate toward the substrate or to be otherwise removed. The fracturable layer is preferably particulate in the various embodiments of the migration imaging members. Such fracturable layers of marking material are typically contiguous to the surface of the softenable layer spaced apart from the substrate, and such fracturable layers

can be substantially or wholly embedded in the softenable layer in various embodiments of the imaging members.

The expression "contiguous" as used herein is intended to mean in actual contact, touching, also, near, though not in contact, and adjoining, and is intended to describe generally the relationship of the fracturable layer of marking material in the softenable layer with the surface of the softenable layer spaced apart from the substrate.

The expression "optically sign-retained" as used herein is intended to mean that the dark (higher optical density) and light (lower optical density) areas of the visible image formed on the migration imaging member correspond to the dark and light areas of the illuminating electromagnetic radiation pattern.

The expression "optically sign-reversed" as used herein is intended to mean that the dark areas of the image formed on the migration imaging member correspond to the light areas of the illuminating electromagnetic radiation pattern and the light areas of the image formed on the migration imaging member correspond to the dark areas of the illuminating electromagnetic radiation pattern.

The expression "optical contrast density" as used herein is intended to mean the difference between maximum optical density ( $D_{max}$ ) and minimum optical density ( $D_{min}$ ) of an image. Optical density is measured for the purpose of this invention by diffuse densitometers with a blue filter which conforms to ANSI PH 2.19 status T response. The expression "optical density" as used herein is intended to mean "transmission optical density" and is represented by the formula:

$$P = \log_{10} (I_s/I)$$

where  $I$  is the transmitted light intensity and  $I_0$  is the incident light intensity. For the purpose of this invention, all values of transmission optical density given in this invention include the substrate density of about 0.2 which is the typical density of a metallized polyester substrate.

High optical density in migration imaging members allows high contrast densities in migration images made from the migration imaging members. High contrast density is highly desirable for most information storage systems. Contrast density is used herein to denote the difference between maximum and minimum optical density in a migration image. The maximum optical density value of an imaged migration imaging member is, of course, the same value as the optical density of an unimaged migration imaging member.

There are various other systems for forming such images, wherein non-photosensitive or inert marking materials are arranged in the aforementioned fracturable layers, or dispersed throughout the softenable layer, as described in the aforementioned patents, which also disclose a variety of methods which can be used to form latent images upon migration imaging members.

Various means for developing the latent images can be used for migration imaging systems. These development methods include solvent wash away, solvent vapor softening, heat softening, and combinations of these methods, as well as any other method which changes the resistance of the softenable material to the migration of particulate marking material through the softenable layer to allow imagewise migration of the particles in depth toward the substrate. In the solvent wash away or meniscus development method, the migration marking material in the light struck region migrates toward the substrate through the softenable layer, which is softened and dissolved, and repacks into a more or less monolayer configuration. In

migration imaging films supported by transparent substrates alone, this region exhibits a maximum optical density which can be as high as the initial optical density of the unprocessed film. On the other hand, the migration marking material in the unexposed region is substantially washed away and this region exhibits a minimum optical density which is essentially the optical density of the substrate alone. Therefore, the image sense of the developed image is optically sign reversed. Various methods and materials and combinations thereof have previously been used to fix such unfixed migration images. One method is to overcoat the image with a transparent abrasion resistant polymer by solution coating techniques. In the heat or vapor softening developing modes, the migration marking material in the light struck region disperses in the depth of the softenable layer after development and this region exhibits  $D_{min}$  which is typically in the range of 0.6 to 0.7. This relatively high  $D_{min}$  is a direct consequence of the depthwise dispersion of the otherwise unchanged migration marking material. On the other hand, the migration marking material in the unexposed region does not migrate and substantially remains in the original configuration, i.e. a monolayer. In migration imaging films supported by transparent substrates, this region exhibits a maximum optical density ( $D_{max}$ ) of about 1.8 to 1.9. Therefore, the image sense of the heat or vapor developed images is optically sign-retained.

Techniques have been devised to permit optically sign-reversed imaging with vapor development, but these techniques are generally complex and require critically controlled processing conditions. An example of such techniques can be found in U.S. Pat. No. 3,795,512, the disclosure of which is totally incorporated herein by reference.

For many imaging applications, it is desirable to produce negative images from a positive original or positive images from a negative original (optically sign-reversing imaging), preferably with low minimum optical density. Although the meniscus or solvent wash away development method produces optically sign-reversed images with low minimum optical density, it entails removal of materials from the migration imaging member, leaving the migration image largely or totally unprotected from abrasion. Although various methods and materials have previously been used to overcoat such unfixed migration images, the post-development overcoating step can be impractically costly and inconvenient for the end users. Additionally, disposal of the effluents washed from the migration imaging member during development can also be very costly.

The background portions of an imaged member can sometimes be transparentized by means of an agglomeration and coalescence effect. In this system, an imaging member comprising a softenable layer containing a fracturable layer of electrically photosensitive migration marking material is imaged in one process mode by electrostatically charging the member, exposing the member to an imagewise pattern of activating electromagnetic radiation, and softening the softenable layer by exposure for a few seconds to a solvent vapor thereby causing a selective migration in depth of the migration material in the softenable layer in the areas which were previously exposed to the activating radiation. The vapor developed image is then subjected to a heating step. Since the exposed particles gain a substantial net charge (typically 85 to 90 percent of the deposited surface charge) as a result of light exposure, they migrate substantially in depth in the softenable layer towards the substrate when exposed to a solvent vapor, thus causing a drastic reduction in optical density. The optical density in this region is

typically in the region of 0.7 to 0.9 (including the substrate density of about 0.2) after vapor exposure, compared with an initial value of 1.8 to 1.9 (including the substrate density of about 0.2). In the unexposed region, the surface charge becomes discharged due to vapor exposure. The subsequent heating step causes the unmigrated, uncharged migration material in unexposed areas to agglomerate or flocculate, often accompanied by coalescence of the marking material particles, thereby resulting in a migration image of very low minimum optical density (in the unexposed areas) in the 0.25 to 0.35 range. Thus, the contrast density of the final image is typically in the range of 0.35 to 0.65. Alternatively, the migration image can be formed by heat followed by exposure to solvent vapors and a second heating step which also results in a migration image with very low minimum optical density. In this imaging system as well as in the previously described heat or vapor development techniques, the softenable layer remains substantially intact after development, with the image being self-fixed because the marking material particles are trapped within the softenable layer.

The word "agglomeration" as used herein is defined as the coming together and adhering of previously substantially separate particles, without the loss of identity of the particles.

The word "coalescence" as used herein is defined as the fusing together of such particles into larger units, usually accompanied by a change of shape of the coalesced particles towards a shape of lower energy, such as a sphere.

Generally, the softenable layer of migration imaging members is characterized by sensitivity to abrasion and foreign contaminants. Since a fracturable layer is located at or close to the surface of the softenable layer, abrasion can readily remove some of the fracturable layer during either manufacturing or use of the imaging member and adversely affect the final image. Foreign contamination such as finger prints can also cause defects to appear in any final image. Moreover, the softenable layer tends to cause blocking of migration imaging members when multiple members are stacked or when the migration imaging material is wound into rolls for storage or transportation. Blocking is the adhesion of adjacent objects to each other. Blocking usually results in damage to the objects when they are separated.

The sensitivity to abrasion and foreign contaminants can be reduced by forming an overcoating such as the overcoatings described in U.S. Pat. No. 3,909,262, the disclosure of which is totally incorporated herein by reference. However, because the migration imaging mechanisms for each development method are different and because they depend critically on the electrical properties of the surface of the softenable layer and on the complex interplay of the various electrical processes involving charge injection from the surface, charge transport through the softenable layer, charge capture by the photosensitive particles and charge ejection from the photosensitive particles, and the like, application of an overcoat to the softenable layer can cause changes in the delicate balance of these processes and result in degraded photographic characteristics compared with the non-overcoated migration imaging member. Notably, the photographic contrast density can degraded. Recently, improvements in migration imaging members and processes for forming images on these migration imaging members have been achieved. These improved migration imaging members and processes are described in U.S. Pat. No. 4,536,458 and U.S. Pat. No. 4,536,457.

Migration imaging members are also suitable for use as masks for exposing the photosensitive material in a printing

plate. The migration imaging member can be laid on the plate prior to exposure to radiation, or the migration imaging member layers can be coated or laminated onto the printing plate itself prior to exposure to radiation, and removed subsequent to exposure.

U.S. Pat. No. 5,102,756 (Vincett et al.), the disclosure of which is totally incorporated herein by reference, discloses a printing plate precursor which comprises a base layer, a layer of photohardenable material, and a layer of softenable material containing photosensitive migration marking material. Alternatively, the precursor can comprise a base layer and a layer of softenable photohardenable material containing photosensitive migration marking material. Also disclosed are processes for preparing printing plates from the disclosed precursors.

U.S. Pat. No. 5,215,838 (Tam et al.), the disclosure of which is totally incorporated herein by reference, discloses a migration imaging member comprising a substrate, an infrared or red light radiation sensitive layer comprising a pigment predominantly sensitive to infrared or red light radiation, and a softenable layer comprising a softenable material, a charge transport material, and migration marking material predominantly sensitive to radiation at a wavelength other than that to which the infrared or red light radiation sensitive pigment is sensitive contained at or near the surface of the softenable layer. When the migration imaging member is imaged and developed, it is particularly suitable for use as a xeroprinting master and can also be used for viewing or for storing data.

U.S. Pat. No. 4,464,450 (Teuscher), the disclosure of which is totally incorporated herein by reference, discloses an electrostatographic imaging member having two electrically operative layers including a charge transport layer and a charge generating layer, the electrically operative layers overlying a siloxane film coated on a metal oxide layer of a metal conductive anode, said siloxane film comprising a reaction product of a hydrolyzed silane having the following general formula:



wherein  $R_1$  is an alkylidene group containing 1 to 20 carbon atoms, and  $R_2$  and  $R_3$  are independently selected from the group consisting of H, a lower alkyl group containing 1 to 3 carbon atoms, a phenyl group, and a poly(ethylene-amino) group, said siloxane having reactive OH and ammonium groups attached to silicon atoms.

c pending application U.S. Ser. No. 08/413,667, now U.S. Pat. No. 5,532,102 filed Mar. 30, 1995, entitled "Improved Apparatus and Process for Preparation of Migration Imaging Members," with the named inventors Philip H. Soden and Arnold L. Pundsack, the disclosure of which is totally incorporated herein by reference, discloses an apparatus for evaporation of a vacuum evaporatable material onto a substrate, said apparatus comprising (a) a walled container for the vacuum evaporatable material having a plurality of apertures in a surface thereof, said apertures being configured so that the vacuum evaporatable material is uniformly deposited onto the substrate; and (b) a source of heat sufficient to effect evaporation of the vacuum evaporatable material from the container through the apertures onto the substrate, wherein the surface of the container having the plurality of apertures therein is maintained at a temperature equal to or greater than the temperature of the vacuum evaporatable material.

Copending application U.S. Ser. No. 08/353,461, now U.S. Pat. No. 5,576,629 filed Dec. 9, 1994, entitled "Improved Migration Imaging Members," with the named inventors Edward G. Zwartz, Carol A. Jennings, Man C. Tam, Philip H. Soden, Arthur Y. Jones, Arnold L. Pundsack, Enrique Levy, Ah-Mee Hor, William W. Limburg, John F. Yanus, Damodar M. Pal, and Dale S. Renfer, the disclosure of which is totally incorporated herein by reference, discloses a migration imaging member comprising a substrate, a first softenable layer comprising a first softenable material and a first migration marking material contained at or near the surface of the first softenable layer spaced from the substrate, and a second softenable layer comprising a second softenable material and a second migration marking material. Also disclosed is a migration imaging process employing the aforesaid imaging member.

Copending application U.S. Ser. No. 08/432,401, now U.S. Pat. No. 5,563,013 filed May 1, 1995, entitled "Pre-Sensitized Infrared or Red Light Sensitive Migration Imaging Members," with the named inventor Man C. Tam, the disclosure of which is totally incorporated herein by reference, discloses a process which comprises (1) providing a migration imaging member comprising a substrate, an infrared or red light radiation sensitive layer comprising a pigment predominantly sensitive to infrared or red light radiation, and a softenable layer comprising a softenable material, a charge transport material, and migration marking material predominantly sensitive to radiation at a wavelength other than that to which the infrared or red light sensitive pigment is predominantly sensitive contained at or near the surface of the softenable layer, said infrared or red light radiation sensitive layer being situated between the substrate and the softenable layer; (2) uniformly charging the imaging member; (3) subsequent to step (2), uniformly exposing the imaging member to activating radiation at a wavelength to which the migration marking material is sensitive; (4) subsequent to step (3), neutralizing charge on the surface of the imaging member spaced from the substrate; (5) subsequent to step (4), exposing the imaging member to infrared or red light radiation at a wavelength to which the infrared or red light radiation sensitive pigment is sensitive in an imagewise pattern, thereby forming an electrostatic latent image on the imaging member, wherein step (5) takes place at least 2 hours after completion of step (4); (6) subsequent to step (5), causing the softenable material to soften, thereby enabling the migration marking material to migrate through the softenable material toward the substrate in an imagewise pattern.

Copending application U.S. Ser. No. 08/432,291, filed May 1, 1995, entitled "Improved Migration Imaging Process," with the named inventors Man C. Tam and Edward G. Zwart, the disclosure of which is totally incorporated herein by reference, discloses a process which comprises (a) providing a migration imaging member comprising (1) a substrate, (2) an infrared or red light radiation sensitive layer comprising a pigment predominantly sensitive to infrared or red light radiation, and (3) a softenable layer comprising a softenable material, a charge transport material, and a photosensitive migration marking material predominantly sensitive to radiation at a wavelength other than that to which the infrared or red light sensitive pigment is predominantly sensitive; (b) uniformly charging the imaging member; (c) subsequent to step (b), uniformly exposing the charged imaging member to a source of activating radiation with a wavelength to which the migration marking material is sensitive, wherein a filter comprising the infrared or red light radiation sensitive pigment is situated between the radiation source and the imaging member; (d) subsequent to step (b),

exposing the imaging member to infrared or red light radiation at a wavelength to which the infrared or red light radiation sensitive pigment is sensitive in an imagewise pattern, thereby forming an electrostatic latent image on the imaging member; and (e) subsequent to steps (c) and (d), causing the softenable material to soften, thereby enabling the migration marking material to migrate through the softenable material toward the substrate in an imagewise pattern.

Copending application U.S. Ser. No. 08/432,448, filed May 1, 1995, entitled "Improved Overcoated Migration Imaging Members," with the named inventors Shadi L. Malhotra and Arthur Y. Jones, the disclosure of which is totally incorporated herein by reference, discloses a migration imaging member comprising (1) a substrate, (2) a softenable layer situated on the substrate, said softenable layer comprising a softenable material and a photosensitive migration marking material, and (3) an overcoating layer situated on the surface of the softenable layer spaced from the substrate, said overcoating layer comprising a material selected from the group consisting of: (a) polyacrylic acids, (b) poly (hydroxyalkylmethacrylates), (c) poly (hydroxyalkylacrylate copolymers, (e) vinyl acetate copolymers, (e) vinyl alcohol-vinyl butyral copolymers, (f) alkyl celluloses, (g) aryl celluloses, (h) hydroxyalkyl cellulose acrylates, (i) hydroxyalkyl cellulose acrylates, (j) hydroxyalkyl cellulose methacrylates, (k) hydroxyaryl cellulose methacrylates, (l) cellulose-acrylamide adducts, (m) poly (vinyl butyral), (n) cyanoethylated celluloses, (o) cellulose acetate hydrogen phthalates, (p) hydroxypropylmethyl cellulose phthalates, (q) hydroxypropyl methyl cellulose succinates, (r) cellulose triacetates, (s) vinyl pyrrolidone-vinyl acetate copolymers, (t) vinyl chloride-vinyl acetate-vinyl alcohol terpolymers, (u) ethylene-maleic anhydride copolymers, (v) styrene-maleic anhydride copolymers, (w) styrene-allyl alcohol copolymers, (x) poly (4-vinylpyridines), (y) polyester latexes, (z) vinyl chloride latexes, (aa) ethylene-vinyl chloride copolymer emulsions, (bb) poly vinyl acetate homopolymer emulsions, (cc) carboxylated vinyl acetate emulsion resins, (dd) vinyl acetate copolymer latexes, (ee) ethylene-vinyl acetate copolymer emulsions, (ff) acrylic-vinyl acetate copolymer emulsions, (gg) vinyl acrylic terpolymer latexes, (hh) acrylic emulsion latexes, (ii) polystyrene latexes, (ii) styrene-butadiene latexes, (kk) butadiene-acrylonitrile latexes, (ll) butadiene-acrylonitrile-styrene terpolymer latexes, (mm) propylene-acrylic acid copolymers, (nn) propylene-ethylene-acrylic acid terpolymers, (oo) poly (vinyl methyl ketones), (pp) poly (trimethyl hexamethylene) terephthalamides, (qq) chlorinated polypropylenes, (rr) poly (hexamethylene sebacates), (ss) poly(ethylene succinates), (tt) poly (caprolactams), (uu) poly (hexamethylene adipamides), (vv) poly (hexamethylene nonaneamides), (ww) poly (hexamethylene sebacamides), (xx) poly (hexamethylene dodecane diamides), (yy) poly (undecanoamides), (zz) poly (lauryllactams), (aaa) ethylene-methacrylic acid ionomers, and (bbb) mixtures thereof.

Copending application U.S. Ser. No. 08/432,380, now U.S. Pat. No. 5,534,374 filed May 1, 1995, entitled "Improved Migration Imaging Members," with the named inventor Shadi L. Malhotra, the disclosure of which is totally incorporated herein by reference, discloses a migration imaging member comprising (a) a substrate, (b) a softenable layer situated on one surface of the substrate, said softenable layer comprising a softenable material and a photosensitive migration marking material, and (c) an antistatic layer situated on the surface of the substrate opposite to the surface in contact with the softenable layer.

Copending application U.S. Ser. No. 08/442,227, now U.S. Pat. No. 5,563,014 filed May 15, 1995, entitled "Improved Migration Imaging Members," with the named inventors Shadi L. Malhotra, Liqin Chen, and Marie-Eve Perron, the disclosure of which is totally incorporated herein by reference, discloses a migration imaging member comprising (a) a substrate, (b) a softenable layer comprising a softenable material and a photosensitive migration marking material, and (c) a transparentizing agent which transparentizes migration marking material in contact therewith contained in at least one layer of the migration imaging member. Also disclosed is a process which comprises (1) providing a migration imaging member comprising (a) a substrate, (b) a softenable layer comprising a softenable material and a photosensitive migration marking material, and (c) a transparentizing agent which transparentizes migration marking material in contact therewith contained in at least one layer of the migration imaging member; (2) uniformly charging the imaging member; (3) subsequent to step (2), exposing the charged imaging member to activating radiation at a wavelength to which the migration marking material is sensitive; (4) subsequent to step (3), causing the softenable material to soften and enabling a first portion of the migration marking material to migrate through the softenable material toward the substrate in an imagewise pattern while a second portion of the migration marking material remains substantially unmigrated within the softenable layer, wherein subsequent to migration of the first portion of migration marking material, either (a) the first portion of migration marking material contacts the transparentizing agent and the second portion of migration marking material does not contact the transparentizing agent; or (b) the second portion of migration marking material contacts the transparentizing agent and the first portion of migration marking material does not contact the transparentizing agent.

Copending application U.S. Ser. No. 08/441,360 now U.S. Pat. No. 5,514,505, filed May 15, 1995, entitled "Method For Obtaining Improved Image Contrast In Migration Imaging Members," with the named inventors William W. Limburg, Joseph Mammino, George Liebermann, Clifford H. Griffiths, Michael M. Shahin, Shadi L. Malhotra, Liqin Chen, and Marie-Eve Perron, the disclosure of which is totally incorporated herein by reference, discloses a process which comprises (a) providing a migration imaging member comprising (1) a substrate and (2) a softenable layer comprising a softenable material and a photosensitive migration marking material present in the softenable layer as a monolayer of particles situated at or near the surface of the softenable layer spaced from the substrate; (b) uniformly charging the imaging member; (3) imagewise exposing the charged imaging member to activating radiation at a wavelength to which the migration marking material is sensitive; (d) subsequent to step (c), causing the softenable material to soften and enabling a first portion of the migration marking material to migrate through the softenable material toward the substrate in an imagewise pattern while a second portion of the migration marking material remains substantially unmigrated within the softenable layer; and (e) contacting the second portion of the migration marking material with a transparentizing agent which transparentizes migration marking material.

Copending application U.S. Ser. No. 08/523,574 now U.S. Pat. No. 5,580,689, filed Sep. 5, 1995, entitled "Improved Migration Imaging Members," with the named inventors Allan K. Chen, Arnold L. Pundsack, Enrique Levy, Eric R. Endrizzi, Richard N. Edwards, Arthur Y. Jones, and Edward G. Zwart, the disclosure of which is totally incor-

porated herein by reference, discloses a migration imaging member comprising a substrate and a softenable layer, said softenable layer comprising a softenable material, a pigment predominantly sensitive to infrared or red light radiation, and a migration marking material predominantly sensitive to radiation at a wavelength other than that to which the infrared or red light radiation sensitive pigment is sensitive contained at least at or near the surface of the softenable layer spaced from the substrate.

Copending application U.S. Ser. No. 08/537,989 now 10 U.S. Pat. No. 5,538,825, filed Oct. 2, 1995, entitled "Printing Plate Preparation Process," with the named inventors Arnold L. Pundsack, Hardy Sonnenberg, and Man C. Tam, the disclosure of which is totally incorporated herein by reference, discloses a process which comprises (a) providing a migration imaging member which comprises a substrate and a softenable layer comprising a softenable material and a photosensitive migration marking material; (b) providing a printing plate precursor which comprises a base layer and a layer of photosensitive material selected from the group consisting of photohardenable materials and photosoftenable materials; (c) placing the softenable layer of the migration imaging member in contact with the layer of photosensitive material of the printing plate precursor and applying heat and pressure to the migration imaging member and printing plate precursor, thereby causing the softenable layer of the migration imaging member to adhere to the layer of photosensitive material of the printing plate precursor; (d) uniformly charging the migration imaging member; (e) subsequent to step (d), exposing the charged imaging member to activating radiation at a wavelength to which the migration marking material is sensitive; (f) subsequent to step (e), causing the softenable material to soften and enabling the migration marking material to migrate through the softenable material in an imagewise pattern, thereby resulting in the layer of softenable material becoming transmissive to light in areas where the migration marking material has migrated and remaining nontransmissive to light in areas where the migration marking material has not migrated; (g) subsequent to step (f), uniformly exposing the migration imaging member and the printing plate precursor to radiation at a wavelength to which the photosensitive material on the printing plate precursor is sensitive, thereby causing the photosensitive material on the printing plate precursor to harden or soften in areas situated contiguous with light-transmissive areas of the softenable layer, thereby forming an imaged printing plate; and (h) subsequent to step (g), removing the migration imaging member from the imaged printing plate.

While known apparatus and processes are suitable for their intended purposes, a need remains for improved migration imaging members. A need further remains for migration imaging members particularly suitable for use as masks for exposing the photosensitive material in a printing plate or a color proofing film. Additionally, there is a need for migration imaging members particularly suitable for use as masks for exposing the photosensitive material in a printing plate or color proofing film with ultraviolet radiation. There is also a need for migration imaging members which enable lowered  $D_{min}$  values. In addition, a need remains for migration imaging members which, when used as masks for exposing the photosensitive material in a printing plate or color proofing film, enable reduced exposure times. Further, a need remains for migration imaging members which, when used as masks for exposing the photosensitive material in a printing plate or color proofing film, enable reduced lamp intensities for exposure. Additionally, a need remains for

migration imaging members having conductive layers with improved uniformity and few or no pinholes (which lead to image defects). There is also a need for migration imaging members which enable uniform  $D_{min}$  values when imaged.

5 There is a further need for migration imaging members which enable color imaging processes that exhibit reduced or no undesirable color shifting. Further, there is a need for migration imaging members which, when placed in stacks or rolls, do not exhibit blocking. Additionally, there is a need for migration imaging members with improved mechanical characteristics. There is also a need for migration imaging members with reduced manufacturing costs. Additionally, a need remains for migration imaging members which exhibit improved adhesion of the softenable layer to the substrate.

#### SUMMARY OF THE INVENTION

It is an object of the present invention to provide migration imaging members with the above noted advantages.

It is another object of the present invention to provide migration imaging members particularly suitable for use as masks for exposing the photosensitive material in a printing plate or a color proofing film.

20 It is yet another object of the present invention to provide migration imaging members particularly suitable for use as masks for exposing the photosensitive material in a printing plate or color proofing film with ultraviolet radiation.

25 It is still another object of the present invention to provide migration imaging members which enable lowered  $D_{min}$  values.

30 Another object of the present invention is to provide migration imaging members which, when used as masks for exposing the photosensitive material in a printing plate or color proofing film, enable reduced exposure times.

35 Yet another object of the present invention is to provide migration imaging members which, when used as masks for exposing the photosensitive material in a printing plate or color proofing film, enable reduced lamp intensities for exposure.

40 Still another object of the present invention is to provide migration imaging members having conductive layers with improved uniformity and few or no pinholes (which lead to image defects).

45 It is another object of the present invention to provide migration imaging members which enable uniform  $D_{min}$  values when imaged.

50 It is yet another object of the present invention to provide migration imaging members which enable color imaging processes that exhibit reduced or no undesirable color shifting.

55 It is still another object of the present invention to provide migration imaging members which, when placed in stacks or rolls, do not exhibit blocking.

Another object of the present invention is to provide migration imaging members with improved mechanical characteristics.

60 Yet another object of the present invention is to provide migration imaging members with reduced manufacturing costs.

It is another object of the present invention to provide migration imaging members which exhibit improved adhesion of the softenable layer to the substrate.

65 These and other objects of the present invention (or specific embodiments thereof) can be achieved by providing a migration imaging member which comprises (a) a

substrate, (b) a conductive layer comprising indium tin oxide dispersed in a polymeric binder, (c) a siloxane film charge blocking layer comprising a hydrolysis reaction product of a silane of the formula



wherein  $\text{R}_1$  is an alkylidene group,  $\text{R}_2$  and  $\text{R}_3$  are each, independent of the other, a hydrogen atom, an alkyl group, a phenyl group, or a poly(ethyleneamino) group, and  $\text{R}_4, \text{R}_5$ , and  $\text{R}_6$  are each, independent of the others, alkyl groups, said siloxane having reactive hydroxyl and ammonium groups attached to silicon atoms, and (d) a softenable layer comprising a softenable material and a photosensitive migration marking material. Optionally an antistatic layer comprising indium tin oxide dispersed in a polymeric binder is situated on the surface of the substrate spaced from the softenable layer.

#### BRIEF DESCRIPTION OF THE DRAWINGS

FIG. 1 illustrates schematically one migration imaging member suitable for the present invention.

FIG. 2 illustrates schematically an infrared or red-light sensitive migration imaging member suitable for the present invention.

FIG. 3 illustrates schematically another infrared or red-light sensitive migration imaging member suitable for the present invention.

#### DETAILED DESCRIPTION OF THE INVENTION

An example of a migration imaging member suitable for the present invention is illustrated schematically in FIG. 1. As illustrated schematically in FIG. 1, migration imaging member 1 comprises a substrate 2, a conductive layer 3 comprising indium tin oxide dispersed in a polymeric binder, an optional adhesive layer 4, a siloxane film charge blocking layer 5, an optional charge transport layer 6, and a softenable layer 7, said softenable layer 7 comprising softenable material 8, migration marking material 9 situated at or near the surface of the layer spaced from the substrate, and optional charge transport material 10 dispersed throughout softenable material 8. Optional overcoating layer 11 is situated on the surface of softenable layer 7 spaced from the substrate 2. Optional antistatic coating 41 is situated on the surface of substrate 2 opposite to that coated with softenable layer 7. Any or all of the optional layers and materials can be absent from the imaging member. In addition, any of the optional layers present need not be in the order shown, but can be in any suitable arrangement. The migration imaging member can be in any suitable configuration, such as a web, a foil, a laminate, a strip, a sheet, a coil, a cylinder, a drum, an endless belt, an endless mobius strip, a circular disc, or any other suitable form.

The substrate can be either electrically conductive or electrically insulating, with transparent materials being preferred. The substrate can be of any suitable material, such as glass, plastic, polyesters such as Mylar® (available from DuPont) or Melinex® 442 (available from ICI Americas, Inc.), polyethylene terephthalate, and the like. The substrate has any effective thickness, typically from about 6 to about 250 microns, and preferably from about 50 to about 200 microns, although the thickness can be outside these ranges.

The conductive layer comprises indium tin oxide dispersed in a polymeric binder. Any suitable or desired binder may be selected. Examples of suitable polymeric binders include gelatin, polyvinyl alcohol, polyvinyl acetate, carboxylated polyvinyl acetate, polyvinyl acetal, polyvinyl chloride, polyvinyl phthalate, polyvinyl methyl ethyl maleic anhydride, polymethylmethacrylate, polyvinyl acetal phthalate, polystyrenebutadiene-acrylonitrile, polyvinyl butyral, polystyrene-maleic acid, polyvinylidene chloride-acrylonitrile, polymethylmethacrylate-methacrylic acid, polybutyl methacrylate-methacrylic acid, cellulose acetate, cellulose acetate-butyrate, cellulose acetate-phthalate, cellulose ethylether phthalate, methylcellulose, ethylcellulose, polymethylacrylate-vinylidene chloride-itaconic acid, poly-2-vinyl pyridine, cellulose acetate diethylamino-acetate, polyvinyl methyl ketone, polyvinyl acetophenone, polyvinyl benzophenone, polyvinylmethyl-acrylate-methacrylic acid, polyvinyl acetate maleic anhydride, polyacrylonitrile acrylic acid, poly-4-vinyl pyridine, carboxylic esters of rosin lactones, polystyrene, cellulose nitrate, polyurethane resins, polyamide resins, phenolic resins, urea resins, melamine resins, ethyl cellulose diethylaminoacetate, other basic polymers, polybasic acid polymers, polyesters, epoxy resins, alkyds, and the like, as well as mixtures thereof. The conductive layer contains indium tin oxide and the polymeric binder in any effective relative amounts. Typically, the indium tin oxide is present in an amount of from about 1 to about 30 percent by weight of the conductive layer, and preferably from about 3 to about 15 percent by weight of the conductive layer, and the binder is present in an amount of from 70 to about 99 percent by weight of the conductive layer, and preferably from about 85 to about 97 percent by weight of the conductive layer, although the amounts can be outside these ranges. Higher amounts of indium tin oxide with respect to the binder will result in greater conductivity of the coating. Indium tin oxide is commercially available, from, for example, Aldrich Chemical Co., Milwaukee, Wis. The conductive layer is of any effective or desired resistance. Typically the resistance of the conductive layer is from about  $5 \times 10^5$  to about  $2 \times 10^{11}$  ohm/cm<sup>2</sup>, and preferably from about  $5 \times 10^5$  to about  $1 \times 10^7$  ohm/cm<sup>2</sup>, although the resistance can be outside this range. The conductive layer is of any suitable or desired thickness; typically the conductive layer has a thickness of from about 0.4 to about 4 microns, and preferably from about 0.4 to about 1 micron, although the thickness can be outside these ranges.

The softenable layer can comprise one or more layers of softenable materials, which can be any suitable material, typically a plastic or thermoplastic material which is soluble in a solvent or softenable, for example, in a solvent liquid, solvent vapor, heat, or any combinations thereof. When the softenable layer is to be softened or dissolved either during or after imaging, it should be soluble in a solvent that does not attack the migration marking material. By softenable is meant any material that can be rendered by a development step as described herein permeable to migration material migrating through its bulk. This permeability typically is achieved by a development step entailing dissolving, melting, or softening by contact with heat, vapors, partial solvents, as well as combinations thereof. Examples of suitable softenable materials include styrene-acrylic copolymers, such as styrene-hexylmethacrylate copolymers, styrene acrylate copolymers, styrene butyl methacrylate copolymers, styrene butylacrylate ethylacrylate copolymers, styrene ethylacrylate acrylic acid copolymers, and the like, polystyrenes, including polyalphamethyl styrene, alkyd substituted polystyrenes, styrene-olefin copolymers, styrenevi-

nyltoluene copolymers, polyesters, polyurethanes, polycarbonates, polyterpenes, silicone elastomers, mixtures thereof, copolymers thereof, and the like, as well as any other suitable materials as disclosed, for example, in U.S. Pat. No. 3,975,195 and other U.S. patents directed to migration imaging members which have been incorporated herein by reference. The softenable layer can be of any effective thickness, typically from about 1 to about 30 microns, preferably from about 2 to about 25 microns, and more preferably from about 2 to about 10 microns, although the thickness can be outside these ranges. The softenable layer can be applied to the conductive layer by any suitable coating process. Typical coating processes include draw bar coating, spray coating, extrusion, dip coating, gravure roll coating, wire-wound rod coating, air knife coating and the like.

The softenable layer also contains migration marking material. The migration marking material can be electrically photosensitive, photoconductive, or of any other suitable combination of materials, or possess any other desired physical property and still be suitable for use in the migration imaging members of the present invention. The migration marking materials preferably are particulate, wherein the particles are closely spaced from each other. Preferred migration marking materials generally are spherical in shape and submicron in size. The migration marking material generally is capable of substantial photodischarge upon electrostatic charging and exposure to activating radiation and is substantially absorbing and opaque to activating radiation in the spectral region where the photosensitive migration marking particles photogenerate charges. The migration marking material is generally present as a thin layer or monolayer of particles situated at or near the surface of the softenable layer spaced from the conductive layer. When present as particles, the particles of migration marking material preferably have an average diameter of up to 2 microns, and more preferably of from about 0.1 to about 1 micron. The layer of migration marking particles is situated at or near that surface of the softenable layer spaced from or most distant from the conductive layer. Preferably, the particles are situated at a distance of from about 0.01 to 0.1 micron from the layer surface, and more preferably from about 0.02 to 0.08 micron from the layer surface. Preferably, the particles are situated at a distance of from about 0.005 to about 0.2 micron from each other, and more preferably at a distance of from about 0.05 to about 0.1 micron from each other, the distance being measured between the closest edges of the particles, i.e. from outer diameter to outer diameter. The migration marking material contiguous to the outer surface of the softenable layer is present in any effective amount, preferably from about 5 to about 80 percent by total weight of the softenable layer, and more preferably from about 25 to about 80 percent by total weight of the softenable layer, although the amount can be outside of this range.

Examples of suitable migration marking materials include selenium, alloys of selenium with alloying components such as tellurium, arsenic, antimony, thallium, bismuth, or mixtures thereof, selenium and alloys of selenium doped with halogens, as disclosed in, for example, U.S. Pat. No. 3,312,548, the disclosure of which is totally incorporated herein by reference, and the like, phthalocyanines, and any other suitable materials as disclosed, for example, in U.S. Pat. No. 3,975,195 and other U.S. patents directed to migration imaging members and incorporated herein reference.

If desired, two or more softenable layers, each containing migration marking particles, can be present in the imaging member as disclosed in copending application U.S. Ser. No.

08/353,461, filed Dec. 9, 1994, entitled "Improved Migration Imaging Members," with the named inventors Edward G. Zwart, Carol A. Jennings, Man C. Tam, Philip H. Soden, Arthur Y. Jones, Arnold L. Pundsack, Enrique Levy, Ah-Mee Hor, William W. Limburg, John F. Yanus, Damodar M. Pal, and Dale S. Renfer, the disclosure of which is totally incorporated herein by reference.

The softenable layer of the migration imaging member optionally contains a charge transport material. The charge transport material can be any suitable charge transport material either capable of acting as a softenable layer material or capable of being dissolved or dispersed on a molecular scale in the softenable layer material. When a charge transport material is also contained in another layer in the imaging member, preferably there is continuous transport of charge through the entire film structure. The charge transport material is defined as a material which is capable of improving the charge injection process for one sign of charge from the migration marking material into the softenable layer and also of transporting that charge through the softenable layer. The charge transport material can be either a hole transport material (transports positive charges) or an electron transport material (transports negative charges). The sign of the charge used to sensitize the migration imaging member during imaging can be of either polarity. Charge transporting materials are well known in the art. Typical charge transporting materials include the following:

Diamine transport molecules of the type described in U.S. Pat. No. 4,306,008, U.S. Pat. No. 4,304,829, U.S. Pat. No. 4,233,384, U.S. Pat. No. 4,115,116, U.S. Pat. No. 4,299,897, and U.S. Pat. No. 4,081,274, the disclosures of each of which are totally incorporated herein by reference. Typical diamine transport molecules include N,N'-diphenyl-N,N'-bis(3'-methylphenyl)-(1,1'-biphenyl)-4,4'-diamine, N,N'-diphenyl-N,N'-bis(4-methylphenyl)-(1,1'-biphenyl)-4,4'-diamine, N,N'-diphenyl-N,N'-bis(2-methylphenyl)-(1,1'-biphenyl)-4,4'-diamine, N,N'-diphenyl-N,N'-bis(3-ethylphenyl)-(1,1'-biphenyl)-4,4'-diamine, N,N'-diphenyl-N,N'-bis(4-ethylphenyl)-(1,1'-biphenyl)-4,4'-diamine, N,N'-diphenyl-N,N'-bis(4-n-butylphenyl)-(1,1'-biphenyl)-4,4'-diamine, N,N'-diphenyl-N,N'-bis(3-chlorophenyl)-(1,1'-biphenyl)-4,4'-diamine, N,N'-diphenyl-N,N'-bis(4-chlorophenyl)-(1,1'-biphenyl)-4,4'-diamine, N,N'-diphenyl-N,N'-bis(phenylmethyl)-(1,1'-biphenyl)-4,4'-diamine, N,N'-N,N'-tetraphenyl-[2,2'-dimethyl-1,1'-biphenyl]-4,4'-diamine, N,N',N',N'-tetra-(4-methylphenyl)-[2,2'-dimethyl-1,1'-biphenyl]-4,4'-diamine, N,N'-diphenyl-N,N'-bis(4-methylphenyl)-[2,2'-dimethyl-1,1'-biphenyl]-4,4'-diamine, N,N'-diphenyl-N,N'-bis(2-methylphenyl)-[2,2'-dimethyl-1,1'-biphenyl]-4,4'-diamine, N,N'-diphenyl-N,N'-bis(3-methylphenyl)-[2,2'-dimethyl-1,1'-biphenyl]-4,4'-diamine, N,N'-diphenyl-N,N'-bis(3-methylphenyl)-pyrenyl-1,6-diamine, and the like.

Pyrazoline transport molecules as disclosed in U.S. Pat. No. 4,315,982, U.S. Pat. No. 4,278,746, and U.S. Pat. No. 3,837,851, the disclosures of each of which are totally incorporated herein by reference. Typical pyrazoline transport molecules include 1-[lepidyl-(2)]-3-(p-diethylaminophenyl)-5-(p-diethylaminophenyl)pyrazoline, 1-[quinolyl-(2)]-3-(p-diethylaminophenyl)-5-(p-diethylaminophenyl)pyrazoline, 1-[pyridyl-(2)]-3-(p-diethylaminophenyl)-5-(p-diethylaminophenyl)pyrazoline, 1-[6-methoxypyridyl-(2)]-3-(p-diethylaminostyryl)-5-(p-diethylaminophenyl)pyrazoline, 1-phenyl-3-[p-diethylaminostyryl]-5-(p-diethylaminostyryl)pyrazoline, 1-phenyl-3-[p-diethylaminostyryl]-5-(p-diethylaminostyryl)pyrazoline, and the like.

Substituted fluorene charge transport molecules as described in U.S. Pat. No. 4,245,021, the disclosure of which is totally incorporated herein by reference. Typical fluorene charge transport molecules include 9-(4'-dimethylaminobenzylidene)fluorene, 9-(4'-methoxybenzylidene)fluorene, 9-(2',4'-dimethoxybenzylidene)fluorene, 2-nitro-9-benzylidene-fluorene, 2-nitro-9-(4'-diethylaminobenzylidene)fluorene, and the like.

Oxadiazole transport molecules such as 2,5-bis(4-diethylaminophenyl)-1,3,4-oxadiazole, pyrazoline, imidazole, triazole, and the like. Other typical oxadiazole transport molecules are described, for example, in German Pat. No. 1,058,836, German Pat. No. 1,060,260, and German Pat. No. 1,120,875, the disclosures of each of which are totally incorporated herein by reference.

Hydrazone transport molecules, such as p-diethylamino benzaldehyde-(diphenylhydrazone), o-ethoxy-p-diethylaminobenzaldehyde-(diphenylhydrazone), o-methyl-p-diethylaminobenzaldehyde-(diphenylhydrazone), o-methyl-p-diethylaminobenzaldehyde-(diphenylhydrazone), 1-naphthalenecarbaldehyde 1-methyl-1-phenylhydrazone, 1-naphthalenecarbaldehyde 1,1-phenylhydrazone, 4-methoxynaphthlene-1-carbaldehyde 1-methyl-1-phenylhydrazone, and the like. Other typical hydrazone transport molecules are described, for example in U.S. Pat. No. 4,150,987, U.S. Pat. No. 4,385,106, U.S. Pat. No. 4,338,388, and U.S. Pat. No. 4,387,147, the disclosures of each of which are totally incorporated herein by reference.

Carbazole phenyl hydrazone transport molecules such as 9-methylcarbazole-3-carbaldehyde-1,1-diphenylhydrazone, 9-ethylcarbazole-3-carbaldehyde-1-methyl-1-phenylhydrazone, 9-ethylcarbazole-3-carbaldehyde-1-ethyl-1-phenylhydrazone, 9-ethylcarbazole-3-carbaldehyde-1-ethyl-1-benzyl-1-phenylhydrazone, 9-ethylcarbazole-3-carbaldehyde-1,1-diphenylhydrazone, and the like. Other typical carbazole phenyl hydrazone transport molecules are described, for example, in U.S. Pat. No. 4,256,821 and U.S. Pat. No. 4,297,426, the disclosures of each of which are totally incorporated herein by reference.

Vinyl-aromatic polymers such as polyvinyl anthracene, polyacenaphthylene; formaldehyde condensation products with various aromatics such as condensates of formaldehyde and 3-bromopyrene; 2,4,7-trinitrofluorenone, and 3,6-dinitro-N-t-butylnaphthalimide as described, for example, in U.S. Pat. No. 3,972,717, the disclosure of which is totally incorporated herein by reference.

Oxadiazole derivatives such as 2,5-bis-(p-diethylaminophenyl)-oxadiazole-1,3,4described in U.S. Pat. No. 3,895,944, the disclosure of which is totally incorporated herein by reference.

Tri-substituted methanes such as alkyl-bis(N,N-dialkylaminoaryl)methane, cycloalkyl-bis(N,N-dialkylaminoaryl)methane, and cycloalkenyl-bis(N,N-dialkylaminoaryl)methane as described in U.S. Pat. No. 3,820,989, the disclosure of which is totally incorporated herein by reference.

9-Fluorenylidene methane derivatives having the formula



10

wherein X and Y are cyano groups or alkoxy carbonyl groups; A, B, and W are electron withdrawing groups independently selected from the group consisting of acyl, alkoxy carbonyl, nitro, alkylaminocarbonyl, and derivatives thereof; m is a number of from 0 to 2; and n is the number 0 or 1 as described in U.S. Pat. No. 4,474,865, the disclosure of which is totally incorporated herein by reference. Typical 9-fluorenylidene methane derivatives encompassed by the above formula include (4-n-butoxycarbonyl-9-fluorenylidene)malononitrile, (4-phenethoxycarbonyl-9-fluorenylidene)malononitrile, (4-carbitoxycarbonyl-9-fluorenylidene)malononitrile, (4-n-butoxycarbonyl-2,7-dinitro-9-fluorenylidene)malonate, and the like.

Other charge transport materials include poly-1-vinylpyrene, poly-9-vinylanthracene, poly-9-(4-pentenyl)-carbazole, poly-9-(5-hexyl)carbazole, polymethylene pyrene, poly-1-(pyrenyl)-butadiene, polymers such as alkyl, nitro, amino, halogen, and hydroxy substitute polymers such as poly-3-amino carbazole, 1,3-dibromo-poly-N-vinyl carbazole, 3,6-dibromo-poly-N-vinyl carbazole, and numerous other transparent organic polymeric or non-polymeric transport materials as described in U.S. Pat. No. 3,870,516, the disclosure of which is totally incorporated herein by reference. Also suitable as charge transport materials are phthalic anhydride, tetrachlorophthalic anhydride, benzil, mellitic anhydride, S-tricyanobenzene, picryl chloride, 2,4-dinitrochlorobenzene, 2,4-dinitrobromobenzene, 4-nitrobiphenyl, 4,4-dinitrophenyl, 2,4,6-trinitroanisole, trichlorotrinitrobenzene, trinitro-O-toluene, 4,6-dichloro-1,3-dinitrobenzene, 4,6-dibromo-1,3-dinitrobenzene, P-dinitrobenzene, chloranil, bromanil, and mixtures thereof, 2,4,7-trinitro-9-fluorenone, 2,4,5,7-tetrinitrofluorenone, trinitroanthracene, dinitroacridene, tetracyanopyrene, dinitroanthraquinone, polymers having aromatic or heterocyclic groups with more than one strongly electron withdrawing substituent such as nitro, sulfonate, carboxyl, cyano, or the like, including polyesters, polysiloxanes, polyamides, polyurethanes, and epoxies, as well as block, graft, or random copolymers containing the aromatic moiety, and the like, as well as mixtures thereof, as described in U.S. Pat. No. 4,081,274, the disclosure of which is totally incorporated herein by reference.

Also suitable are charge transport materials such as triarylamines, including trityl amine, of the formula



55

60

65

and the like, as disclosed in, for example, U.S. Pat. No. 3,240,597 and U.S. Pat. No. 3,180,730, the disclosures of

which are totally incorporated herein by reference, and substituted diarylmethane and triarylmethane compounds, including bis-(4-diethylamino-2-methylphenyl)phenylmethane, of the formula



and the like, as disclosed in, for example, U.S. Pat. No. 4,082,551, U.S. Pat. No. 3,755,310, U.S. Pat. No. 3,647,431, British Patent 984,965, British Patent 980,879, and British Patent 1,141,666, the disclosure of which are totally incorporated herein by reference.

When the charge transport molecules are combined with an insulating binder to form the softenable layer, the amount of charge transport molecule which is used can vary depending upon the particular charge transport material and its compatibility (e.g. solubility) in the continuous insulating film forming binder phase of the softenable matrix layer and the like. Satisfactory results have been obtained using between about 5 percent to about 50 percent by weight charge transport molecule based on the total weight of the softenable layer. A particularly preferred charge transport molecule is one having the general formula



wherein X, Y and Z are selected from the group consisting of hydrogen, an alkyl group having from 1 to about 20 carbon atoms and chlorine, and at least one of X, Y and Z is independently selected to be an alkyl group having from 1 to about 20 carbon atoms or chlorine. If Y and Z are hydrogen, the compound can be named N,N'-diphenyl-N,N'-bis(alkylphenyl)-[1,1'-biphenyl]-4,4'-diamine wherein the alkyl is, for example, methyl, ethyl, propyl, n-butyl, or the like, or the compound can be N,N'-diphenyl-N,N'-bis(chlorophenyl)-[1,1'-biphenyl]-4,4'-diamine. Results can be obtained when the softenable layer contains between about 8 percent to about 40 percent by weight of these diamine compounds based on the total weight of the softenable layer. Optimum results are achieved when the softenable layer contains between about 16 percent to about 32 percent by weight of N,N'-diphenyl-N,N'-bis(3"-methylphenyl)-(1,1'-biphenyl)-4,4'-diamine based on the total weight of the softenable layer.

The charge transport material is present in the softenable material in any effective amount, typically from about 5 to about 50 percent by weight and preferably from about 8 to about 40 percent by weight, although the amount can be outside these ranges. Alternatively, the softenable layer can employ the charge transport material as the softenable material if the charge transport material possesses the nec-

essary film-forming characteristics and otherwise functions as a softenable material. The charge transport material can be incorporated into the softenable layer by any suitable technique. For example, it can be mixed with the softenable layer components by dissolution in a common solvent. If desired, a mixture of solvents for the charge transport material and the softenable layer material can be employed to facilitate mixing and coating. The charge transport molecule and softenable layer mixture can be applied to the substrate by any conventional coating process. Typical coating processes include draw bar coating, spray coating, extrusion, dip coating, gravure roll coating, wire-wound rod coating, air knife coating, and the like.

The optional adhesive layer can include any suitable adhesive material. Typical adhesive materials include copolymers of styrene and an acrylate, polyester resin such as DuPont 49000 (available from E. I. duPont de Nemours Company), copolymer of acrylonitrile and vinylidene chloride, polyvinyl acetate, polyvinyl butyral and the like and mixtures thereof. The adhesive layer can have any thickness, typically from about 0.05 to about 1 micron, although the thickness can be outside of this range. When an adhesive layer is employed, it preferably forms a uniform and continuous layer having a thickness of about 0.5 micron or less to ensure satisfactory discharge during the imaging process. It can also optionally include charge transport molecules.

The optional charge transport layer can comprise any suitable film forming binder material. Typical film forming binder materials include styrene acrylate copolymers, polycarbonates, co-polycarbonates, polyesters, co-polyesters, polyurethanes, polyvinyl acetate, polyvinyl butyral, polystyrenes, alkyd substituted polystyrenes, styrene-olefin copolymers, styrene-co-n-hexylmethacrylate, an 80/20 mole percent copolymer of styrene and hexylmethacrylate having an intrinsic viscosity of 0.179 dl/gm; other copolymers of styrene and hexylmethacrylate, styrene-vinyltoluene copolymers, polyalpha-methylstyrene, mixtures thereof, and copolymers thereof. The above group of materials is not intended to be limiting, but merely illustrative of materials suitable as film forming binder materials in the optional charge transport layer. The film forming binder material typically is substantially electrically insulating and does not adversely chemically react during the imaging process. Although the optional charge transport layer has been described as coated on a substrate, in some embodiments, the charge transport layer itself can have sufficient strength and integrity to be substantially self supporting and can, if desired, be brought into contact with a suitable conductive substrate during the imaging process.

As is well known in the art, a uniform deposit of electrostatic charge of suitable polarity can be substituted for a conductive layer. Alternatively, a uniform deposit of electrostatic charge of suitable polarity on the exposed surface of the charge transport spacing layer can be substituted for a conductive layer to facilitate the application of electrical migration forces to the migration layer. This technique of "double charging" is well known in the art. The charge transport layer is of any effective thickness, typically from about 1 to about 25 microns, and preferably from about 2 to about 20 microns, although the thickness can be outside these ranges.

Charge transport molecules suitable for the charge transport layer are described in detail hereinabove. The specific charge transport molecule utilized in the charge transport layer of any given imaging member can be identical to or different from the charge transport molecule employed in the adjacent softenable layer. Similarly, the concentration of the

charge transport molecule utilized in the charge transport spacing layer of any given imaging member can be identical to or different from the concentration of charge transport molecule employed in the adjacent softenable layer. When the charge transport material and film forming binder are combined to form the charge transport spacing layer, the amount of charge transport material used can vary depending upon the particular charge transport material and its compatibility (e.g. solubility) in the continuous insulating film forming binder. Satisfactory results have been obtained using between about 5 percent and about 50 percent based on the total weight of the optional charge transport spacing layer, although the amount can be outside this range. The charge transport material can be incorporated into the charge transport layer by techniques similar to those employed for the softenable layer.

The charge blocking layer comprises a siloxane or hydrolyzed silane having the general formula



or



or mixtures thereof, wherein  $\text{R}_1$  is an alkylidene group, preferably with from 1 to about 20 carbon atoms,  $\text{R}_2$  and  $\text{R}_3$  are each, independent of the other, a hydrogen atom, an alkyl group, preferably with from 1 to about 3 carbon atoms, a phenyl group, or a poly(ethylene-amino) group,  $\text{R}_7$  is a hydrogen atom, an alkyl group, preferably with from 1 to about 3 carbon atoms, or a phenyl group,  $\text{X}^{\ominus}$  is an anion from an acid or acidic salt,  $n$  is 1, 2, 3, or 4, and  $y$  is 1, 2, 3, or 4. The material is formed by hydrolyzing a hydrolyzable silane having the general formula



wherein  $\text{R}_1$  is an alkylidene group, preferably with from 1 to about 20 carbon atoms,  $\text{R}_2$  and  $\text{R}_3$  are each, independent of the other, a hydrogen atom, an alkyl group, preferably with from 1 to about 3 carbon atoms, a phenyl group, or a poly(ethylene-amino) group, and  $\text{R}_4$ ,  $\text{R}_5$ , and  $\text{R}_6$  are each, independent of the others, alkyl groups, preferably with from 1 to about 4 carbon atoms. Examples of hydrolyzable silanes include 3-aminopropyl triethoxy silane, N-aminoethyl-3-aminopropyl trimethoxy silane, 3-aminopropyl trimethoxy silane, (N,N'-dimethyl-3-amino) propyl triethoxysilane, (N,N'-diethyl-3-amino) propyl trimethoxysilane, N,N'-dimethylamino phenyl triethoxy silane, N-phenyl aminopropyl trimethoxy silane, N-methyl aminopropyl trimethoxy silane, trimethoxy silylpropyl-diethylene triamine, bis (2-hydroxyethyl) aminopropyl triethoxy silane, N-trimethoxysilyl propyl-N,N-dimethyl ammonium acetate, N-trimethoxysilylpropyl-N,N,N-

trimethyl chloride, and the like. Specific examples of materials suitable for the charge blocking layer include 3-aminopropyl triethoxy silane (gamma APS), 3-aminopropyl trimethoxy silane, both available from Aldrich Chemical Co., Milwaukee, Wis., and the like. Further information regarding charge blocking materials of this type is disclosed in, for example, U.S. Pat. No. 4,464,450, the disclosure of which is totally incorporated herein by reference.

The silane is hydrolyzed by admixing the silane with sufficient water to hydrolyze the alkoxy groups attached to the silicon atom. The aqueous solution formed thereby can be coated onto the imaging member. Preferred solutions contain from about 0.05 to about 1.5 percent by weight silane, although the amount can be outside this range. The solution preferably is maintained at a pH of from about 4 to about 10. Preferred reaction temperatures are from about 100° to about 150° C., although the temperature can be outside this range. The hydrolyzed silane can also be applied to the migration imaging member in another solvent, such as 20 methanol, ethanol, water, or the like, as well as mixtures thereof.

Any desired or suitable technique can be used to apply the hydrolyzed silane solution to the imaging member. Typical application techniques include draw bar coating, spray 25 coating, extrusion, dip coating, gravure roll coating, wire-wound rod coating, air knife coating, and the like. Alternatively, the unhydrolyzed silane can be applied to the imaging member, followed by hydrolysis of the silane by any desired method, such as treatment with water vapor or 30 the like. Drying of the hydrolyzed silane preferably is carried out at temperatures above room temperature. After drying, the siloxane reaction product film formed from the hydrolyzed silane contains larger molecules, in which  $n$  is equal to or greater than 6; the reaction product of the hydrolyzed 35 silane may be linear, partially crosslinked, a dimer, a trimer, or the like. The charge blocking layer is of any effective thickness, typically from about 0.005 to about 2 microns, and preferably from about 0.025 to about 1 micron, although the thickness can be outside these ranges.

As illustrated schematically in FIG. 2, migration imaging member 21 comprises in the order shown a substrate 22, a conductive layer 23 comprising indium tin oxide dispersed in a polymeric binder, an optional adhesive layer 24, a siloxane film charge blocking layer 25, an optional charge 40 transport layer 26, a softenable layer 27, said softenable layer 27 comprising softenable material 28, charge transport material 29, and migration marking material 30 situated at or near the surface of the layer spaced from the substrate, and an infrared or red light radiation sensitive layer 31 situated 45 on softenable layer 27 comprising infrared or red light radiation sensitive pigment particles 32 optionally dispersed in polymeric binder 33. Alternatively (not shown), infrared or red light radiation sensitive layer 31 can comprise infrared or red light radiation sensitive pigment particles 32 directly deposited as a layer by, for example, vacuum evaporation techniques or other coating methods. Optional overcoating layer 34 is situated on the surface of imaging member 21 spaced from the substrate 22. Optional antistatic layer 35 is situated on the surface of substrate 22 opposite to 50 that coated with softenable layer 27.

As illustrated schematically in FIG. 3, migration imaging member 41 comprises in the order shown a substrate 42, a conductive layer 43 comprising indium tin oxide dispersed in a polymeric binder, an optional adhesive layer 44, a siloxane film charge blocking layer 45, an infrared or red light radiation sensitive layer 46 comprising infrared or red 55 light radiation sensitive pigment particles 47 optionally

dispersed in polymeric binder 48, an optional charge transport layer 49, and a softenable layer 50, said softenable layer 50 comprising softenable material 51, charge transport material 52, and migration marking material 53 situated at or near the surface of the layer spaced from the substrate. Optional overcoating layer 54 is situated on the surface of imaging member 41 spaced from the substrate 42. Optional antistatic layer 55 is situated on the surface of substrate 42 opposite to that coated with softenable layer 50.

The infrared or red light sensitive layer generally comprises a pigment sensitive to infrared and/or red light radiation. While the infrared or red light sensitive pigment may exhibit some photosensitivity in the wavelength to which the migration marking material is sensitive, it is preferred that photosensitivity in this wavelength range be minimized so that the migration marking material and the infrared or red light sensitive pigment exhibit absorption peaks in distinct, different wavelength regions. This pigment can be deposited as the sole or major component of the infrared or red light sensitive layer by any suitable technique, such as vacuum evaporation or the like. An infrared or red light sensitive layer of this type can be formed by placing the pigment and the imaging member comprising the substrate and any previously coated layers into an evacuated chamber, followed by heating the infrared or red light sensitive pigment to the point of sublimation. The sublimed material recondenses to form a solid film on the imaging member. Alternatively, the infrared or red light sensitive pigment can be dispersed in a polymeric binder and the dispersion coated onto the imaging member to form a layer. Examples of suitable red light sensitive pigments include perylene pigments such as benzimidazole perylene, dibromoanthrone, crystalline trigonal selenium, beta-metal free phthalocyanine, azo pigments, and the like, as well as mixtures thereof. Examples of suitable infrared sensitive pigments include X-metal free phthalocyanine, metal phthalocyanines such as vanadyl phthalocyanine, chloroiridium phthalocyanine, titanyl phthalocyanine, chloroaluminum phthalocyanine, copper phthalocyanine, magnesium phthalocyanine, and the like, squaraines, such as hydroxy squaraine, and the like as well as mixtures thereof. Examples of suitable optional polymeric binder materials include polystyrene, styrene-acrylic copolymers, such as styrene-hexamethacrylate copolymers, styrene-vinyl toluene copolymers, polyesters, such as PE-200, available from Goodyear, polyurethanes, polyvinylcarbazoles, epoxy resins, phenoxy resins, polyamide resins, polycarbonates, polyterpenes, silicone elastomers, polyvinylalcohols, such as Gelvatol 20-90, 9000, 20-60, 6000, 20-30, 3000, 40-20, 40-10, 26-90, and 30-30, available from Monsanto Plastics and Resins Co., St. Louis, Mo., polyvinylformals, such as Formvar 12/85, 5/95E, 6/95E, 7/95E, and 15/95E, available from Monsanto Plastics and Resins Co., St. Louis, Mo., polyvinylbutyrals, such as Butvar B-72, B-74, B-73, B-76, B-79, B-90, and B-98, available from Monsanto Plastics and Resins Co., St. Louis, Mo., Zeneca resin A622, available from Zeneca Colours, Wilmington, Del., and the like as well as mixtures thereof. When the infrared or red light sensitive layer comprises both a polymeric binder and the pigment, the layer typically comprises the binder in an amount of from about 5 to about 95 percent by weight and the pigment in an amount of from about 5 to about 95 percent by weight, although the relative amounts can be outside this range. Preferably, the infrared or red light sensitive layer comprises the binder in an amount of from about 40 to about 90 percent by weight and the pigment in an amount of from about 10 to about 60 percent by weight. Optionally, the infrared

sensitive layer can contain a charge transport material as described herein when a binder is present; when present, the charge transport material is generally contained in this layer in an amount of from about 5 to about 30 percent by weight of the layer. The optional charge transport material can be incorporated into the infrared or red light radiation sensitive layer by any suitable technique. For example, it can be mixed with the infrared or red light radiation sensitive layer components by dissolution in a common solvent. If desired, a mixture of solvents for the charge transport material and the infrared or red light sensitive layer material can be employed to facilitate mixing and coating. The infrared or red light radiation sensitive layer mixture can be applied to the substrate by any conventional coating process. Typical coating processes include draw bar coating, spray coating, extrusion, dip coating, gravure roll coating, wire-wound rod coating, air knife coating, and the like. An infrared or red light sensitive layer wherein the pigment is present in a binder can be prepared by dissolving the polymer binder in a suitable solvent, dispersing the pigment in the solution by ball milling, coating the dispersion onto the imaging member comprising the substrate and any previously coated layers, and evaporating the solvent to form a solid film. When the infrared or red light sensitive layer is coated directly onto the softenable layer containing migration marking material, preferably the selected solvent is capable of dissolving the polymeric binder for the infrared or red sensitive layer but does not dissolve the softenable polymer in the layer containing the migration marking material. One example of a suitable solvent is isobutanol with a polyvinyl butyral binder in the infrared or red sensitive layer and a styrene/ethyl acrylate/acrylic acid terpolymer softenable material in the layer containing migration marking material. The infrared or red light sensitive layer can be of any effective thickness. Typical thicknesses for infrared or red light sensitive layers comprising a pigment and a binder are from about 0.05 to about 2 microns, and preferably from about 0.1 to about 1.5 microns, although the thickness can be outside these ranges. Typical thicknesses for infrared or red light sensitive layers consisting of a vacuum-deposited layer of pigment are from about 200 to about 2,000 Angstroms, and preferably from about 300 to about 1,000 Angstroms, although the thickness can be outside these ranges.

The optional overcoating layer can be substantially electrically insulating, or have any other suitable properties. The overcoating preferably is substantially transparent, at least in the spectral region where electromagnetic radiation is used for imagewise exposure steps in the imaging process. The overcoating layer is continuous and preferably of a thickness up to about 3 microns. More preferably, the overcoating has a thickness of between about 0.5 and about 2 microns to minimize residual charge buildup. Overcoating layers greater than about 3 microns thick can also be used. Typical overcoating materials include acrylic-styrene copolymers, methacrylate polymers, methacrylate copolymers, styrene-butylmethacrylate copolymers, butylmethacrylate resins, vinylchloride copolymers, fluorinated homo or copolymers, high molecular weight polyvinyl acetate, organosilicon polymers and copolymers, polyesters, polycarbonates, polyamides, polyvinyl toluene and the like. The overcoating layer generally protects the softenable layer to provide greater resistance to the adverse effects of abrasion during handling and imaging. The overcoating layer preferably adheres strongly to the softenable layer to minimize damage. The overcoating layer can also have adhesive properties at its outer surface which provide improved resistance to toner

filming during toning, transfer, and/or cleaning. The adhesive properties can be inherent in the overcoating layer or can be imparted to the overcoating layer by incorporation of another layer or component of adhesive material. These adhesive materials should not degrade the film forming components of the overcoating and preferably have a surface energy of less than about 20 ergs/cm<sup>2</sup>. Typical adhesive materials include fatty acids, salts and esters, fluorocarbons, silicones, and the like. The coatings can be applied by any suitable technique such as draw bar, spray, dip, melt, extrusion or gravure coating. It will be appreciated that these overcoating layers protect the imaging member before imaging, during imaging, and after the members have been imaged.

The optional antistatic layer generally comprises a binder and an antistatic agent. The binder and antistatic agent are present in any effective relative amounts, typically from about 1 to about 30 percent by weight antistatic agent and from about 70 to about 99 percent by weight binder, although the relative amounts can be outside this range. Typical thicknesses for the antistatic layer are from about 0.4 to about 2 microns, and preferably from about 0.4 to about 1 micron, although the thickness can be outside these ranges. The antistatic layer can be applied to the imaging member by any desired method, such as draw bar coating, spray coating, extrusion, dip coating, gravure roll coating, wire-wound rod coating, air knife coating, and the like. In one preferred method, the antistatic layer is coated onto the imaging member by a slot extrusion process, wherein a flat die is situated with the die lips in close proximity to the web of the substrate to be coated, resulting in a continuous film of the coating solution evenly distributed across followed by drying sheet, followed by drying in an air dryer at 100° C.

Any suitable or desired binder can be employed. Examples of suitable binders include (a) hydrophilic polysaccharides and their modifications, such as (1) starch (such as starch SLS-280, available from St. Lawrence starch), (2) cationic starch (such as Cato-72, available from National Starch), (3) hydroxyalkylstarch, wherein alkyl has at least one carbon atom and wherein the number of carbon atoms is such that the material is water soluble, preferably from about 1 to about 20 carbon atoms, and more preferably from about 1 to about 10 carbon atoms, such as methyl, ethyl, propyl, butyl, or the like (such as hydroxypropyl starch (#02382, available from Poly Sciences inc.) and hydroxyethyl starch (#06733, available from Poly Sciences Inc.)), (4) gelatin (such as Calfskin gelatin #00639, available from Poly Sciences Inc.), (5) alkyl celluloses and aryl celluloses, wherein alkyl has at least one carbon atom and wherein the number of carbon atoms is such that the material is water soluble, preferably from 1 to about 20 carbon atoms, more preferably from 1 to about 10 carbon atoms, and even more preferably from 1 to about 7 carbon atoms, such as methyl, ethyl, propyl, butyl, pentyl, hexyl, benzyl, and the like (such as methyl cellulose (Methocel AM 4, available from Dow Chemical Company)), and wherein aryl has at least 6 carbon atoms and wherein the number of carbon atoms is such that the material is water soluble, preferably from 6 to about 20 carbon atoms, more preferably from 6 to about 10 carbon atoms, and even more preferably about 6 carbon atoms, such as phenyl, (6) hydroxy alkyl celluloses, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, pentyl, hexyl, benzyl, or the like (such as hydroxyethyl cellulose (Natrosol 250 LR, available from

Hercules Chemical Company), and hydroxypropyl cellulose (Klucel Type E, available from Hercules Chemical Company)), (7) alkyl hydroxy alkyl celluloses, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, pentyl, hexyl, benzyl, or the like (such as ethyl hydroxyethyl cellulose (Bermocoll, available from Berol Kem. A. B. Sweden)), (8) hydroxy alkyl alkyl celluloses, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as hydroxyethyl methyl cellulose (HEM, available from British Celanese Ltd., also available as Tylose MH, MHK from Kalle A. G.)), hydroxypropyl methyl cellulose (Methocel K35LV, available from Dow Chemical Company), and hydroxy butylmethyl cellulose (such as HBMC, available from Dow Chemical Company)), (9) dihydroxyalkyl cellulose, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as dihydroxypropyl cellulose, which can be prepared by the reaction of 3-chloro-1,2-propane with alkali cellulose), (10) hydroxy alkyl hydroxy alkyl cellulose, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as hydroxypropyl hydroxyethyl cellulose, available from Aqualon Company), (11) halodeoxycellulose, wherein halo represents a halogen atom (such as chlorodeoxycellulose, which can be prepared by the reaction of cellulose with sulfonyl chloride in pyridine at 25° C.), (12) amino deoxycellulose (which can be prepared by the reaction of chlorodeoxy cellulose with 19 percent alcoholic solution of ammonia for 6 hours at 160° C.), (13) dialkylammonium halide hydroxy alkyl cellulose, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, and wherein halide represents a halogen atom (such as diethylammonium chloride hydroxy ethyl cellulose, available as Celquat H-100, L-200, National Starch and Chemical Company), (14) hydroxyalkyl trialkyl ammonium halide hydroxyalkyl cellulose, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, and wherein halide represents a halogen atom (such as hydroxypropyl trimethyl ammonium chloride hydroxyethyl cellulose, available from Union Carbide Company as Polymer JR), (15) dialkyl amino alkyl cellulose, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, (such as diethyl amino ethyl cellulose, available from Poly Sciences Inc. as DEAE cellulose #05178), (16) carboxyalkyl dextrans, wherein alkyl has at least one carbon atom and

wherein the number of carbon atoms is such that the material is water soluble, preferably from 1 to about 20 carbon atoms, more preferably from 1 to about 10 carbon atoms, such as methyl, ethyl, propyl, butyl, pentyl, hexyl, and the like, (such as carboxymethyl dextrans, available from Poly Sciences Inc. as #16058), (17) dialkyl aminoalkyl dextran, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as diethyl aminoethyl dextran, available from Poly Sciences Inc. as #5178), (18) amino dextran (available from Molecular Probes Inc), (19) carboxy alkyl cellulose salts, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, and wherein the cation is any conventional cation, such as sodium, lithium, potassium, calcium, magnesium, or the like (such as sodium carboxymethyl cellulose CMC 7HOF, available from Hercules Chemical Company), (20) gum arabic (such as #G9752, available from Sigma Chemical Company), (21) carrageenan (such as #C1013 available from Sigma Chemical Company), (22) Karaya gum (such as #G0503, available from Sigma Chemical Company), (23) xanthan (such as Keltrol-T, available from Kelco division of Merck and Company), (24) chitosan (such as #C3646, available from Sigma Chemical Company), (25) carboxy-alkyl hydroxyalkyl guar, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as carboxymethyl hydroxypropyl guar, available from Auqualon Company), (26) cationic guar (such as Celanese Jaguars C-14-S, C-15, C-17, available from Celanese Chemical Company), (27) n-carboxyalkyl chitin, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, such as n-carboxymethyl chitin, (28) dialkyl ammonium hydrolyzed collagen protein, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like (such as dimethyl ammonium hydrolyzed collagen protein, available from Croda as Croquats), (29) agar-agar (such as that available from Pfaltz and Bauer Inc), (30) cellulose sulfate salts, wherein the cation is any conventional cation, such as sodium, lithium, potassium, calcium, magnesium, or the like (such as sodium cellulose sulfate #023 available from Scientific Polymer Products), and (31) carboxyalkylhydroxyalkyl cellulose salts, wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl and the like, and wherein the cation is any conventional cation, such as sodium, lithium, potassium, calcium, magnesium, or the like (such as sodium carboxymethylhydroxyethyl cellulose CMHEC 43H and 37L available from Hercules Chemical Company); (b) vinyl polymers, such as (1) poly(vinyl alcohol) (such as Elvanol available from Dupont Chemical Company), (2) poly(vinyl

phosphate) (such as #4391 available from Poly Sciences Inc.), (3) poly (vinyl pyrrolidone) (such as that available from GAF Corporation), (4) vinyl pyrrolidone-vinyl acetate copolymers (such as #02587, available from Poly Sciences Inc.), (5) vinyl pyrrolidone-styrene copolymers (such as #371, available from Scientific Polymer Products), (6) poly (vinylamine) (such as #1562, available from Poly Sciences Inc.), (7) poly (vinyl alcohol) alkoxylated, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as poly (vinyl alcohol) ethoxylated #6573, available from Poly Sciences Inc.), and (8) poly (vinyl pyrrolidone-dialkylaminoalkyl alkylacrylate), wherein each alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as poly (vinyl pyrrolidone-diethylaminomethylmethacrylate) #16294 and #16295, available from Poly Sciences Inc.); (c) formaldehyde resins, such as (1) melamine-formaldehyde resin (such as BC 309, available from British Industrial Plastics Limited), (2) urea-formaldehyde resin (such as BC777, available from British Industrial Plastics Limited), and (3) alkylated urea-formaldehyde resins, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as methylated urea-formaldehyde resins, available from American Cyanamid Company as Beetle 65); (d) ionic polymers, such as (1) poly (2-acrylamido-2-methyl propane sulfonic acid) (such as #175 available from Scientific Polymer Products), (2) poly (N,N-dimethyl-3,5-dimethylene piperidinium chloride) (such as #401, available from Scientific Polymer Products), and (3) poly (methylene-guanidine) hydrochloride (such as #654, available from Scientific Polymer Products); (e) latex polymers, such as (1) cationic, anionic, and nonionic styrene-butadiene latexes (such as that available from Gen Corp Polymer Products, such as RES 4040 and RES 4100, available from Unocal Chemicals, and such as DL 6672A, DL6638A, and DL6663A, available from Dow Chemical Company), (2) ethylene-vinylacetate latex (such as Airflex 400, available from Air Products and Chemicals Inc.), (3) vinyl acetate-acrylic copolymer latexes (such as synthemul 97-726, available from Reichhold Chemical Inc, Resyn 25-1110 and Resyn 25-1140, available from National Starch Company, and RES 3103 available from Unocal Chemicals; (4) quaternary acrylic copolymer latexes, particularly those of the formula



wherein n is a number from about 10 to about 100, and preferably about 50, R is hydrogen or methyl, R<sub>1</sub> is hydrogen, an alkyl group, or an aryl group, and R<sub>2</sub> is N+(CH<sub>3</sub>)<sub>3</sub>X<sup>-</sup>, wherein X is an anion, such as Cl, Br, I, HSO<sub>3</sub>, SO<sub>3</sub>, CH<sub>3</sub>SO<sub>3</sub>, H<sub>2</sub>PO<sub>4</sub>, HPO<sub>4</sub>, PO<sub>4</sub>, or the like, and the degree of quaternization is from about 1 to about 100 percent, including polymers such as polymethyl acrylate trimethyl ammonium chloride latex, such as HX42-1, available from Interpolymer Corp., or the like; (f) maleic anhydride and maleic acid containing polymers, such as (1)

styrene-maleic anhydride copolymers (such as that available as Scriptet from Monsanto, and the SMA series available from Arco), (2) vinyl alkyl ether-maleic anhydride copolymers, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as vinyl methyl ether-maleic anhydride copolymer #173, available from Scientific Polymer Products), (3) alkylene-maleic anhydride copolymers, wherein alkylene has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as ethylene-maleic anhydride copolymer #2308, available from Poly Sciences Inc., also available as EMA from Monsanto Chemical Company), (4) butadiene-maleic acid copolymers (such as #07787, available from Poly Sciences Inc.), (5) vinylalkylether-maleic acid copolymers, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as vinylmethylether-maleic acid copolymer, available from GAF Corporation as Gantrez S-95), and (6) alkyl vinyl ether-maleic acid esters, wherein alkyl has at least one carbon atom and wherein the number of carbon atoms is such that the material is water soluble, preferably from 1 to about 20 carbon atoms, more preferably from 1 to about 10 carbon atoms, such as methyl, ethyl, propyl, butyl, and the like (such as methyl vinyl ether-maleic acid ester #773, available from Scientific Polymer Products); (g) acrylamide containing polymers, such as (1) poly (acrylamide) (such as #02806, available from Poly Sciences Inc.), (2) acrylamide-acrylic acid copolymers (such as #04652, #02220, and #18545, available from Poly Sciences Inc.), and (3) poly (N,N-dimethyl acrylamide) (such as #004590, available from Poly Sciences Inc.); and (h) poly (alkylene imine) containing polymers, wherein alkylene has two (ethylene), three (propylene), or four (butylene) carbon atoms, such as (1) poly(ethylene imine) (such as #135, available from Scientific Polymer Products), (2) poly (ethylene imine) epichlorohydrin (such as #634, available from Scientific Polymer Products), and (3) alkoxylated poly (ethylene imine), wherein alkyl has one (methoxylated), two (ethoxylated), three (propoxylated), or four (butoxylated) carbon atoms (such as ethoxylated poly (ethylene imine) #636, available from Scientific Polymer Products); and the like. Any mixtures of the above ingredients in any relative amounts can also be employed.

Any desired or suitable antistatic agent can be employed. Indium tin oxide is a particularly preferred antistatic agent.

In one particularly preferred embodiment of the present invention, the migration imaging member is prepared with a substrate which comprises a polyester (such as ICI 054 or ICI 454) with a thickness of about 4.0 mils and is coated on both surfaces with conductive layers each having a thickness of from about 0.4 to about 1 micron and comprising indium tin oxide dispersed in a binder. This three layered article is available from Arkwright Inc., Fiskeville, R.I., as SUPER CLEAR 106. The three-layered article is then coated on one surface with the softenable layer (and any other desired optional layers), with the exposed surface of the three-layered article subsequent to coating functioning as an antistatic layer. The resistance of SUPER CLEAR 106 is generally from about  $3 \times 10^6$  to about  $5 \times 10^6$  ohm/cm<sup>2</sup>.

Imaging members of the present invention are exposed and developed by known processes, such as those disclosed in, for example, U.S. Pat. No. 5,215,838 (Tam et al.), the disclosure of which is totally incorporated herein by reference. In one embodiment of the present invention the imaging member can be developed by a process which comprises uniformly charging the imaging member, exposing the charged member to activating radiation at a wavelength to which the migration marking material is sensitive in an imagewise pattern, thereby forming an electrostatic latent image on the imaging member, and thereafter causing the softenable material to soften, thereby enabling the migration marking material to migrate through the softenable material toward the substrate in an imagewise pattern. In embodiments of the present invention wherein the migration imaging member contains an infrared or red light sensitive material, the member can be developed by a process which comprises uniformly charging the imaging member, exposing the charged imaging member to infrared or red light radiation at a wavelength to which the infrared or red light radiation sensitive pigment is sensitive in an imagewise pattern, thereby forming an electrostatic latent image on the imaging member, uniformly exposing the imaging member to activating radiation at a wavelength to which the migration marking material is sensitive, and causing the softenable material to soften, thereby enabling the migration marking material to migrate through the softenable material toward the substrate in an imagewise pattern.

In a preferred embodiment, the present invention includes an imaging process which comprises (1) providing a migration imaging member which comprises (a) a substrate, (b) a conductive layer comprising indium tin oxide dispersed in a polymeric binder, (c) a siloxane film charge blocking layer, and (d) a softenable layer comprising a softenable material and a photosensitive migration marking material; (2) uniformly charging the migration imaging member; (3) exposing the charged migration imaging member to a source of activating radiation in an imagewise pattern; (4) causing the softenable material to soften, thereby enabling the migration marking material to migrate through the softenable material toward the conductive layer in an imagewise pattern; (5) providing a printing plate precursor which comprises a base layer and a layer of photosensitive material selected from the group consisting of photohardenable materials and photosoftenable materials; and (6) exposing the printing plate precursor and the migration imaging member wherein the migration marking material has migrated toward the substrate in an imagewise fashion to radiation at a wavelength to which the photosensitive material on the printing plate precursor is sensitive, wherein substantially all of the radiation to which the printing plate precursor is exposed passes first through the migration imaging member, thereby causing the photosensitive material on the printing plate precursor to harden or soften in areas situated contiguous with light-transmissive areas of the migration imaging member, thereby forming an imaged printing plate. In a particularly preferred embodiment, the printing plate precursor is exposed to radiation at a wavelength in the ultraviolet wavelength range, specifically from about 300 to about 500 nanometers. Examples of suitable printing plate materials and configurations are disclosed in, for example, U.S. Pat. No. 5,102,756 (Vincett et al.), the disclosure of which is totally incorporated herein by reference.

In another preferred embodiment, the present invention includes an imaging process which comprises (1) providing a migration imaging member which comprises (a) a substrate, (b) a conductive layer comprising indium tin

oxide dispersed in a polymeric binder, (c) a siloxane film charge blocking layer, and (d) a softenable layer comprising a softenable material and a photosensitive migration marking material; (2) uniformly charging the migration imaging member; (3) exposing the charged migration imaging member to a source of activating radiation in an imagewise pattern; (4) causing the softenable material to soften, thereby enabling the migration marking material to migrate through the softenable material toward the conductive layer in an imagewise pattern; (5) providing a photosensitive film; and (6) exposing the photosensitive film and the migration imaging member wherein the migration marking material has migrated toward the substrate in an imagewise fashion to radiation at a wavelength to which the photosensitive material on the printing plate precursor is sensitive, wherein substantially all of the radiation to which the photosensitive film is exposed passes first through the migration imaging member, thereby forming an image on the photosensitive film. In a particularly preferred embodiment, the photosensitive film is exposed to radiation at a wavelength in the ultraviolet wavelength range, specifically from about 300 to about 500 nanometers.

Specific embodiments of the invention will now be described in detail. These examples are intended to be illustrative, and the invention is not limited to the materials, conditions, or process parameters set forth in these embodiments. All parts and percentages are by weight unless otherwise indicated.

#### EXAMPLE I

A 4 mil thick polyester sheet (ICI 454) measuring 6 inches×12.5 inches was coated on both sides with indium tin oxide dispersed in a polymeric binder (Super Clear 106, obtained from Arkwright Inc.). The film exhibited a resistivity of  $3.5 \times 10^6$  ohms per square centimeter. Thereafter a charge blocking layer was applied to one of the conductive indium tin oxide layers by coating one surface of the sheet with a solution containing 2.5 percent by weight hydrolyzed 3-aminopropyltriethoxysilane in a solvent mixture of ethanol and n-heptane (solvent containing 75 percent by weight ethanol and 25 percent by weight n-heptane) using a CSD draw down table and a Consler coating rod #10. The wet film was then mounted on an aluminum heat block set to 100° C. for 60 seconds to dry. Subsequently a solution containing 15 percent by weight of a terpolymer of styrene/ethylacrylate/acrylic acid (prepared as disclosed in U.S. Pat. No. 4,853,307, the disclosure of which is totally incorporated herein by reference) in toluene was coated on the charge blocking layer using a CSD draw down table and a Consler coating rod #10. The deposited softenable layer was allowed to dry at about 115° C. for about 2 minutes, resulting in a dried softenable layer with a thickness of about 4 microns. Onto a donor sheet of 3 mil thick polyester (Melinex 442, obtained from Imperial Chemical Industries (ICI), aluminized to 20 percent light transmission) was coated a solution containing 15 percent by weight of a terpolymer of styrene/ethylacrylate/acrylic acid (prepared as disclosed in U.S. Pat. No. 4,853,307, the disclosure of which is totally incorporated herein by reference) in toluene using a CSD draw down table and a Consler coating rod #10. The deposited softenable layer was allowed to dry at about 115° C. for about 2 minutes, resulting in a dried softenable layer with a thickness of about 4 microns. Thereafter, the temperature of the softenable layers on the imaging member and on the donor sheet were raised to about 115° C. to lower the viscosity of the exposed surfaces of the softenable layers to about  $5 \times 10^3$  poises in preparation for the deposition of

marking material. Thin layers of particulate vitreous selenium were then applied by vacuum deposition in a vacuum chamber maintained at a vacuum of about  $4 \times 10^{-4}$  Torr. The imaging member and the donor sheet were then rapidly chilled to room temperature. Reddish monolayers of selenium particles having an average diameter of about 0.3 micron embedded about 0.05 to 0.1 micron below the surfaces of the copolymer layers were formed. The selenium-coated softenable layer of the imaging member was then placed in contact with the selenium-coated softenable layer on the donor sheet, and the "sandwich" thus formed was fed between the two heated pressure rollers in an AGFA ADL 45 laminator. The heater in the laminator was set to 100° C., and the measured surface temperature of the top and bottom rollers was 80° to 85° C. The roller speed was 50 centimeters per minute. Thereafter, when the laminated imaging member had cooled to room temperature, the aluminized polyester donor sheet was peeled from the member at a 180 degree angle using a continuous smooth motion, resulting in formation of an imaging member having two softenable layers containing migration marking material.

The migration imaging member thus prepared was then uniformly placed on a charge table ( $I_{table} = 40 \mu A$ ) moving at 88 inches per minute and grounded with copper tape. The imaging member was negatively charged to a surface voltage of -625 V with a corona charging device set at -6.1 KV and set at a height of 6.3 millimeters at a temperature between 21° and 24° C.; a relative humidity of 23 to 33 percent, and with room lights off and red safe lights on. The charged member was subsequently optically exposed by placing a test pattern mask comprising a UGRA 1982 target silver halide image in contact with the imaging member in a small vacuum frame to hold the target mask in intimate contact with the member and exposing the member to blue light of 480 nanometers through the mask for a period of 6 seconds. The exposed imaging member was then developed by subjecting it to a temperature of 115° C. for 5 seconds using a small aluminum heating block in contact with the surface of the sheet spaced from the softenable layer. The optical density of the imaging member in the  $D_{max}$  and  $D_{min}$  area were measured using a MacBeth TR927 densitometer. The blue setting corresponds to a Wratten No. 47 filter and the ultraviolet setting corresponds to a Wratten No. 18A filter. The film exhibited a  $D_{min}$  of 0.75 and an optical contrast of 2.08 for blue, and a  $D_{min}$  of 0.75 and an optical contrast of 2.03 for UV light. The image was also assessed using a 10×loupe, and the resulting images were of high quality.

#### EXAMPLE II

The procedure of Example I was repeated with the exception that no charge blocking layer was applied to the imaging member. The film exhibited a  $D_{min}$  of 2.35 and an optical contrast of 0.67 for blue, and a  $D_{min}$  of 2.28 and an optical contrast of 0.68 for UV light.

#### EXAMPLE III

The procedure of Example I was repeated with the exception that the siloxane charge blocking layer was replaced with a charge blocking layer applied by coating a solution containing 5 percent by weight gelatin from swine skin in water. The film exhibited a  $D_{min}$  of 0.77 and an optical contrast of 2.16 for blue, and  $D_{min}$  of 0.77 and an optical contrast of 2.02 for UV light. The film had very poor mechanical properties as a result of poor adhesion of the gelatin charge blocking layer to the substrate.

## EXAMPLE IV

The procedure of Example I was repeated with the exception that the siloxane charge blocking layer was replaced with a charge blocking layer applied by coating a solution containing 5 percent by weight (poly(2-hydroxyethylmethacrylate) in methanol. The film exhibited a  $D_{min}$  of 2.69 and an optical contrast of 0.35 for blue, and a  $D_{min}$  of 2.59 and an optical contrast of 0.29 for UV light.

## EXAMPLE V

The procedure of Example I was repeated with the exception that the siloxane charge blocking layer was replaced with a charge blocking layer applied by coating a solution containing 5 percent by weight poly(vinyl acetate) in methanol. The film exhibited a  $D_{min}$  of 2.75 and an optical contrast of 0.27 for blue, and a  $D_{min}$  of 2.66 and an optical contrast of 0.27 for UV light.

## EXAMPLE VI

The procedure of Example I was repeated with the exception that the siloxane charge blocking layer was replaced with a charge blocking layer applied by coating a solution containing 5 percent by weight (poly(2-hydroxypropylmethacrylate) in methanol. The film exhibited a  $D_{min}$  of 2.60 and an optical contrast of 0.41 for blue, and a  $D_{min}$  of 2.53 and an optical contrast of 0.38 for UV light.

## EXAMPLE VII

The procedure of Example I was repeated with the exception that no softenable layer was solution coated onto the charge blocking layer. Instead, a softenable layer was applied to a first donor sheet by the procedure described in Example I. A second donor sheet was then placed in contact with the selenium-coated softenable layer on the first donor sheet and the "sandwich" thus formed was passed through the laminator, followed by removal of the first donor sheet. The second donor sheet was then placed in contact with the charge blocking layer of the imaging member and the "sandwich" thus formed was passed through the laminator, followed by removal of the second donor sheet, resulting in formation of an imaging member having a single softenable layer with selenium particles situated at or near the surface of the softenable layer spaced from the charge blocking layer. The film exhibited a  $D_{min}$  of 0.53 and an optical contrast of 0.95 for blue, and a  $D_{min}$  of 0.53 and an optical contrast of 0.83 for UV light.

## EXAMPLE VIII

The procedure of Example I was repeated with the exception that subsequent to application of the siloxane charge blocking layer, a pigment dispersion was prepared by ball milling for 24 hours a mixture comprising 10.6 parts by weight solids in an n-butyl acetate solvent, wherein the solids comprised 5 percent by weight X-metal-free phthalocyanine (prepared as described in U.S. Pat. No. 3,357,989, the disclosure of which is totally incorporated by reference) and 95 percent by weight of an ethylene vinyl acetate/vinyl chloride-vinyl acetate copolymer. The resulting dispersion was hand coated onto the charge blocking layer of the migration imaging member with a #5 Meyer rod, followed by drying the deposited infrared-sensitive layer at 50° C. for 1 minute by contacting the substrate to an aluminum heating block. The two softenable layers each contained about 76 percent by weight of the terpolymer and about 24 percent by

weight of a tritylamine charge transfer material prior to vacuum evaporation of the selenium particles onto the softenable layers. The film exhibited a  $D_{min}$  of 0.80 and an optical contrast of 2.20 for blue, and a  $D_{min}$  of 0.87 and an optical contrast of 1.95 for UV light.

## EXAMPLE IX

The procedure of Example I was repeated with the exception that the indium tin oxide coated substrate was replaced with a substrate comprising 4 mil polyester film (ICI 454) coated with copper iodide. No image was obtained subsequent to exposure and development.

## EXAMPLE X

The procedure of Example I was repeated with the exception that the indium tin oxide coated substrate was replaced with a substrate comprising 4 mil polyester film (ICI 454) coated with copper iodide and the siloxane charge blocking layer was replaced with a charge blocking layer applied by coating a solution containing 5 percent by weight (poly(2-hydroxyethylmethacrylate) in methanol. The film exhibited a  $D_{min}$  of 1.79 and an optical contrast of 0.21 for blue, and a  $D_{min}$  of 1.72 and an optical contrast of 0.23 for UV light.

## EXAMPLE XI

Antistatic tests were performed on a migration imaging member prepared as described in Example I and, for comparison purposes, on a migration imaging member prepared as described in Example I with the exception that the indium tin oxide coating was applied only to one surface of the polyester substrate, followed by coating the indium tin oxide layer with the charge blocking and softenable layers, resulting in formation of a migration imaging member having no indium tin oxide antistatic coating on the surface of the substrate spaced from the softenable layer. The tests were performed using a Princeton Electro Dynamics 276A Static Charge Analyzer. The imaging member without an antistatic coating was charged up to 1,020 volts, and the imaging member retained the charge without decay in 60 seconds. The imaging member with the indium tin oxide antistatic coating was able to be charged to only 50 volts, and decayed to about zero volts in 25 seconds.

## EXAMPLE XII

Blocking tests were performed on a migration imaging member prepared as described in Example I and, for comparison purposes, on migration imaging members prepared as described in Example I with the exception that the indium tin oxide coating was applied only to one surface of the polyester substrate and the other surface of the polyester substrate was coated with an antistatic layer comprising a quaternary ammonium salt in a quaternary acrylic copolymer latex binder (relative amounts about 15 percent by weight quaternary ammonium salt and about 85 percent by weight binder). The quaternary ammonium salts used were ammonium chloride, ammonium bromide, and ammonium iodide. The blocking tests were performed on stacks of five 1 inch×1 inch samples of the migration imaging members under the following conditions: 20° C. at 50% relative humidity; 20° C. at 80% relative humidity; 45° C. at 50% relative humidity; and 45° C. at 80% relative humidity. These conditions represent standard storage conditions for migration imaging members, and also represent extreme conditions to which the film may be exposed. The imaging

member samples were conditioned under these conditions in a Hotpack Temperature-Humidity Chamber for a period of 24 hours. Thereafter, the sample sets were placed between the jaw of a TWN-16 Super Pillow Block, which was placed inside of the Temperature-Humidity Chamber, and pressed for 24 hours at pressures of 2.6, 5.1, 10.5, and 21.5 kilograms per square inch. The imaging members with the indium tin oxide antistatic coating passed all of these tests without any coating separation from substrate, whereas the imaging members with quaternary ammonium salts as anti-static coating all exhibited significant blocking; transfer of large patches of the antistatic layer of one member to the softenable layer of the adjacent member in the stack was observed for these imaging members containing the quaternary ammonium salt antistatic layers.

#### EXAMPLE XIII

Migration imaging members prepared as described in Example I were tested for imaging performance. Three stacks each containing five 2.0"×13" portions of the member were placed between two pieces of polished metal plates (2.5"×13.5"). Pressures of 1.15, 2.5 and 3.7 kilograms per square inch were applied to the stacks for 24 hours. No transfer of antistatic coatings to the softenable layers was observed. Thereafter, the imaging members were charged, exposed, and developed as described in Example I. The imaged members each exhibited a  $D_{min}$  of 0.75 and an optical contrast of 2.15 for blue light, and a  $D_{min}$  of 0.75 and an optical contrast of 2.12 for UV light. The same test was performed on an infrared-sensitive migration imaging member prepared as described in Example VIII. The imaging results were equivalent to those in Example VIII. No adverse effects were caused by antistatic coating. After the imaging process, no scratches or fingerprints were observed.

Other embodiments and modifications of the present invention may occur to those skilled in the art subsequent to a review of the information presented herein; these embodiments and modifications, as well as equivalents thereof, are also included within the scope of this invention.

What is claimed is:

1. A migration imaging member which comprises (a) a substrate, (b) a conductive layer comprising indium tin oxide dispersed in a polymeric binder, (c) a siloxane film charge blocking layer comprising a hydrolysis reaction product of a silane of the formula



wherein  $R_1$  is an alkylidene group,  $R_2$  and  $R_3$  are each, independent of the other, a hydrogen atom, an alkyl group, a phenyl group, or a poly(ethylene-amino) group, and  $R_4, R_5$ , and  $R_6$  are each, independent of the others, alkyl groups, said siloxane having reactive hydroxyl and ammonium groups attached to silicon atoms, and (d) a softenable layer comprising a softenable material and a photosensitive migration marking material.

2. A migration imaging member according to claim 1 wherein the conductive layer has a thickness of from about 0.4 to about 4 microns.

3. A migration imaging member according to claim 1 wherein the conductive layer has a thickness of from about 0.4 to about 1 micron.

4. A migration imaging member according to claim 1 wherein the indium tin oxide is present in the conductive layer in an amount of from about 1 to about 30 percent by weight.

5. A migration imaging member according to claim 1 wherein the indium tin oxide is present in the conductive layer in an amount of from about 3 to about 15 percent by weight.

6. A migration imaging member according to claim 1 wherein the charge blocking layer has a thickness of from about 0.005 to about 2 microns.

7. A migration imaging member according to claim 1 wherein the charge blocking layer has a thickness of from about 0.025 to about 1 micron.

8. A migration imaging member according to claim 1 wherein  $R_1$  is an alkylidene group with from 1 to about 20 carbon atoms,  $R_2$  and  $R_3$  are each, independent of the other, a hydrogen atom, an alkyl group with from 1 to about 3 carbon atoms, a phenyl group, or a poly(ethylene-amino) group, and  $R_4, R_5$ , and  $R_6$  are each, independent of the others, alkyl groups with from 1 to about 4 carbon atoms.

9. A migration imaging member according to claim 1 wherein the siloxane is selected from the group consisting of (a) those of the formula



20 (b) those of the formula



25 and (c) mixtures thereof, wherein  $R_1$  is an alkylidene group,  $R_2$  and  $R_3$  are each, independent of the other, a hydrogen atom, an alkyl group, a phenyl group, or a poly(ethylene-amino) group,  $R_7$  is a hydrogen atom, an alkyl group, or a phenyl group,  $X$  is an anion from an acid or acidic salt,  $n$  is 1, 2, 3, or 4, and  $y$  is 1, 2, 3, or 4.

30 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 94

14. A migration imaging member according to claim 1 further comprising an antistatic layer comprising indium tin oxide dispersed in a polymeric binder situated on the surface of the substrate spaced from the softenable layer.

**15.** A migration imaging member according to claim 14 wherein the antistatic layer has a thickness of from about 0.4 to about 2 microns.

**16. A migration imaging member according to claim 14 wherein the antistatic layer has a thickness of from about 0.4 to about 1 micron.**

17. A migration imaging member according to claim 14 wherein the indium tin oxide is present in the antistatic layer in an amount of from about 1 to about 30 percent by weight.

18. A migration imaging member according to claim 14 wherein the indium tin oxide is present in the antistatic layer in an amount of from about 3 to about 15 percent by weight.

in an amount of from about 5 to about 15 percent by weight.

**19.** A migration imaging member according to claim 1 wherein the imaging member also comprises a second softenable layer containing a second softenable material, a second migration marking material, and an optional charge transport material.

**20.** An imaging process which comprises (1) providing a migration imaging member which comprises (a) a substrate, (b) a conductive layer comprising indium tin oxide dispersed in a polymeric binder, (c) a siloxane film charge blocking layer comprising a hydrolysis reaction product of a silane of the formula



wherein  $R_1$  is an alkylidene group,  $R_2$  and  $R_3$  are each, independent of the other, a hydrogen atom, an alkyl group, a phenyl group, or a poly(ethylene-amino) group, and  $R_4, R_5$ , and  $R_6$  are each, independent of the others, alkyl groups, said siloxane having reactive hydroxyl and ammonium groups attached to silicon atoms, and (d) a softenable layer comprising a softenable material and a photosensitive migration marking material; (2) uniformly charging the migration imaging member; (3) exposing the charged migration imaging member to a source of activating radiation in an imagewise pattern; (4) causing the softenable material to soften, thereby enabling the migration marking material to migrate through the softenable material toward the conductive layer in an imagewise pattern; (5) providing a printing plate precursor which comprises a base layer and a layer of photosensitive material selected from the group consisting of photohardenable materials and photosoftenable materials; and (6) exposing the printing plate precursor and the migration imaging member wherein the migration marking material has migrated toward the substrate in an imagewise

fashion to radiation at a wavelength to which the photosensitive material on the printing plate precursor is sensitive, wherein substantially all of the radiation to which the printing plate precursor is exposed passes first through the migration imaging member, thereby causing the photosensitive material on the printing plate precursor to harden or soften in areas situated contiguous with light-transmissive areas of the migration imaging member, thereby forming an imaged printing plate.

10 21. An imaging process according to claim 20 wherein the printing plate precursor is exposed to radiation at a wavelength of from about 300 to about 500 nanometers.

22. An imaging process which comprises (1) providing a migration imaging member which comprises (a) a substrate, 15 (b) a conductive layer comprising indium tin oxide dispersed in a polymeric binder, (c) a siloxane film charge blocking layer comprising a hydrolysis reaction product of a silane of the formula



25 wherein  $R_1$  is an alkylidene group,  $R_2$  and  $R_3$  are each, independent of the other, a hydrogen atom, an alkyl group, a phenyl group, or a poly(ethylene-amino) group, and  $R_4$ ,  $R_5$ , and  $R_6$  are each, independent of the others, alkyl groups, said siloxane having reactive hydroxyl and ammonium groups attached to silicon atoms, and (d) a softenable layer comprising a softenable material and a photosensitive migration marking material; (2) uniformly charging the migration imaging member; (3) exposing the charged migration imaging member to a source of activating radiation in an imagewise pattern; (4) causing the softenable material to soften, thereby enabling the migration marking material to migrate through the softenable material toward the conductive layer in an imagewise pattern; (5) providing a photosensitive film; and (6) exposing the photosensitive film and the migration imaging member wherein the migration marking material has migrated toward the substrate in an imagewise fashion to radiation at a wavelength to which the photosensitive material on the printing plate precursor is sensitive, wherein substantially all of the radiation to which the photosensitive film is exposed passes first through the migration imaging member, thereby forming an image on the photosensitive film.

50 23. An imaging process according to claim 22 wherein the photosensitive film is exposed to radiation at a wavelength of from about 300 to about 500 nanometers.

• • • • •